



US011753599B2

(12) **United States Patent**  
Shao et al.

(10) **Patent No.:** US 11,753,599 B2  
(45) **Date of Patent:** Sep. 12, 2023

|                                                                                                                                                                                        |                |         |                                  |
|----------------------------------------------------------------------------------------------------------------------------------------------------------------------------------------|----------------|---------|----------------------------------|
| (54) <b>LUBRICATING COMPOSITIONS FOR A HYBRID ENGINE</b>                                                                                                                               | 4,261,843 A    | 4/1981  | King et al.                      |
| (71) Applicant: <b>AFTON CHEMICAL CORPORATION</b> , Richmond, VA (US)                                                                                                                  | 4,263,152 A    | 4/1981  | King et al.                      |
| (72) Inventors: <b>Huifang Shao</b> , Moseley, VA (US); <b>Mark Devlin</b> , Glen Allen, VA (US); <b>Paul Ransom</b> , Huddersfield (GB); <b>Guillaume Carpentier</b> , Bracknell (GB) | 4,265,773 A    | 5/1981  | deVries et al.                   |
| (73) Assignee: <b>AFTON CHEMICAL CORPORATION</b> , Richmond, VA (US)                                                                                                                   | 4,272,387 A    | 6/1981  | King et al.                      |
| (*) Notice: Subject to any disclaimer, the term of this patent is extended or adjusted under 35 U.S.C. 154(b) by 0 days.                                                               | 4,283,295 A    | 8/1981  | deVries et al.                   |
|                                                                                                                                                                                        | 4,285,822 A    | 8/1981  | deVries et al.                   |
|                                                                                                                                                                                        | 4,963,275 A    | 10/1990 | Gutierrez et al.                 |
|                                                                                                                                                                                        | 4,971,711 A    | 11/1990 | Lundberg et al.                  |
|                                                                                                                                                                                        | 5,241,003 A    | 8/1993  | Degonia et al.                   |
|                                                                                                                                                                                        | 5,650,381 A    | 7/1997  | Gatto et al.                     |
|                                                                                                                                                                                        | RE37,363 E     | 9/2001  | Gatto et al.                     |
|                                                                                                                                                                                        | 6,300,291 B1   | 10/2001 | Hartley et al.                   |
|                                                                                                                                                                                        | 6,327,852 B1   | 12/2001 | Hirose                           |
|                                                                                                                                                                                        | 6,425,365 B1   | 7/2002  | Peters et al.                    |
|                                                                                                                                                                                        | 6,723,685 B2   | 4/2004  | Hartley et al.                   |
|                                                                                                                                                                                        | 6,769,400 B1   | 8/2004  | Ament                            |
|                                                                                                                                                                                        | 6,856,034 B2   | 2/2005  | Peters et al.                    |
|                                                                                                                                                                                        | 6,958,409 B1 * | 10/2005 | Ruhe, Jr. .... C07F 9/17 508/379 |
| (21) Appl. No.: <b>17/662,420</b>                                                                                                                                                      | RE38,929 E     | 1/2006  | Gatto et al.                     |
| (22) Filed: <b>May 6, 2022</b>                                                                                                                                                         | 7,059,306 B2   | 6/2006  | Reddy                            |
| (65) <b>Prior Publication Data</b>                                                                                                                                                     | 7,214,649 B2   | 5/2007  | Loper et al.                     |
| US 2022/0389345 A1 Dec. 8, 2022                                                                                                                                                        | 7,373,917 B2   | 5/2008  | Ellinger et al.                  |
|                                                                                                                                                                                        | 7,395,659 B2   | 7/2008  | Pott                             |

(Continued)

**FOREIGN PATENT DOCUMENTS**

|    |              |        |
|----|--------------|--------|
| CN | 104560297 B9 | 3/2013 |
| CN | 104334697 A  | 2/2015 |

(Continued)

**OTHER PUBLICATIONS**

Lubes'N'Greases, "EV Lubricant Technology" Perspective on Electric Vehicles, LNG Publishing Company (2019): 1-13.  
 Lubes'N'Greases, "Perspective on Electric Vehicles." 2019 Annual Report, LNG Publishing Company (2019): 1-74.  
 Extended European Search Report for corresponding European application No. 22175318.9; dated Oct. 20, 2022 (8 pages).

|                                                                                                                                                                                                                                                                                                                                                                                             |           |
|---------------------------------------------------------------------------------------------------------------------------------------------------------------------------------------------------------------------------------------------------------------------------------------------------------------------------------------------------------------------------------------------|-----------|
| (51) <b>Int. Cl.</b>                                                                                                                                                                                                                                                                                                                                                                        |           |
| <i>C10M 137/10</i>                                                                                                                                                                                                                                                                                                                                                                          | (2006.01) |
| <i>C10M 125/10</i>                                                                                                                                                                                                                                                                                                                                                                          | (2006.01) |
| <i>C10M 133/16</i>                                                                                                                                                                                                                                                                                                                                                                          | (2006.01) |
| <i>C10M 169/04</i>                                                                                                                                                                                                                                                                                                                                                                          | (2006.01) |
| <i>C10N 10/04</i>                                                                                                                                                                                                                                                                                                                                                                           | (2006.01) |
| <i>C10N 20/02</i>                                                                                                                                                                                                                                                                                                                                                                           | (2006.01) |
| <i>C10N 30/04</i>                                                                                                                                                                                                                                                                                                                                                                           | (2006.01) |
| <i>C10N 30/06</i>                                                                                                                                                                                                                                                                                                                                                                           | (2006.01) |
| <i>C10N 40/25</i>                                                                                                                                                                                                                                                                                                                                                                           | (2006.01) |
| (52) <b>U.S. Cl.</b>                                                                                                                                                                                                                                                                                                                                                                        |           |
| CPC ..... <i>C10M 137/10</i> (2013.01); <i>C10M 125/10</i> (2013.01); <i>C10M 133/16</i> (2013.01); <i>C10M 169/04</i> (2013.01); <i>C10M 2201/062</i> (2013.01); <i>C10M 2215/086</i> (2013.01); <i>C10M 2223/045</i> (2013.01); <i>C10N 2010/04</i> (2013.01); <i>C10N 2020/02</i> (2013.01); <i>C10N 2030/04</i> (2013.01); <i>C10N 2030/06</i> (2013.01); <i>C10N 2040/25</i> (2013.01) |           |

|                                                                                                                                                                                                                                          |  |
|------------------------------------------------------------------------------------------------------------------------------------------------------------------------------------------------------------------------------------------|--|
| (58) <b>Field of Classification Search</b>                                                                                                                                                                                               |  |
| CPC ..... C10M 137/10; C10M 125/10; C10M 133/16; C10M 169/04; C10M 2201/062; C10M 2215/086; C10M 2223/045; C10M 2215/28; C10M 2219/046; C10N 2010/04; C10N 2020/02; C10N 2030/04; C10N 2030/06; C10N 2040/25; C10N 2030/38; C10N 2030/50 |  |

See application file for complete search history.

**References Cited****U.S. PATENT DOCUMENTS**

|             |        |                |
|-------------|--------|----------------|
| 4,259,194 A | 3/1981 | deVries et al. |
| 4,259,195 A | 3/1981 | King et al.    |

**11 Claims, No Drawings**

The present disclosure relates to methods for improving phosphorus retention and improving antiwear performance in an internal combustion engine of a hybrid vehicle, comprising lubricating the internal combustion engine of the hybrid vehicle with a lubricating oil composition comprising: greater than 50 wt. % of a base oil of lubricating viscosity; and an amount of one or more zinc dialkyl dithiophosphate compound(s) sufficient to provide: from about 100 ppmw phosphorus to about 1000 ppmw phosphorus, based on a total weight of the lubricating oil composition; and from about 10 ppmw zinc to about 1200 ppmw zinc, based on the total weight of the lubricating oil composition.

| (56)                  | References Cited |                    |                          |                 |                      |                   |
|-----------------------|------------------|--------------------|--------------------------|-----------------|----------------------|-------------------|
| U.S. PATENT DOCUMENTS |                  |                    |                          |                 |                      |                   |
| 7,448,367 B1          | 11/2008          | Reddy et al.       | 2018/0030866 A1          | 2/2018          | Blasinski            |                   |
| RE40,595 E            | 12/2008          | Gatto et al.       | 2018/0079990 A1          | 3/2018          | Aoyama               |                   |
| 7,607,293 B2          | 10/2009          | Tamai et al.       | 2018/0100114 A1          | 4/2018          | Gao et al.           |                   |
| 7,645,726 B2          | 1/2010           | Loper              | 2018/0100115 A1          | 4/2018          | Gao et al.           |                   |
| 7,732,390 B2          | 6/2010           | Kadkhodayan et al. | 2018/0100117 A1          | 4/2018          | Flores-Torres et al. |                   |
| 7,954,579 B2          | 6/2011           | Rodriguez et al.   | 2018/0100118 A1          | 4/2018          | Flores-Torres et al. |                   |
| 8,039,976 B2          | 10/2011          | Sato et al.        | 2018/0100120 A1          | 4/2018          | Flores-Torres et al. |                   |
| 8,048,831 B2          | 11/2011          | Loper              | 2018/0113058 A1          | 4/2018          | Schroder et al.      |                   |
| 8,090,520 B2          | 1/2012           | Tate, Jr. et al.   | 2018/0134983 A1          | 5/2018          | Broutin et al.       |                   |
| 8,251,022 B2          | 8/2012           | Yaccarino          | 2018/0258365 A1          | 9/2018          | Ohkubo et al.        |                   |
| 8,322,472 B2          | 12/2012          | Gonze              | 2018/0258366 A1 *        | 9/2018          | Ohkubo .....         | C10M 169/04       |
| 8,400,030 B1          | 3/2013           | Tang et al.        | 2018/0265075 A1          | 9/2018          | Kamatani et al.      |                   |
| 8,459,007 B2          | 6/2013           | Maier et al.       | 2019/0039594 A1          | 2/2019          | Luehrs et al.        |                   |
| 8,578,914 B2          | 11/2013          | Lee et al.         | 2019/0106651 A1          | 4/2019          | Kubo et al.          |                   |
| 8,627,654 B2          | 1/2014           | Roos et al.        | 2019/0118793 A1          | 4/2019          | Jang                 |                   |
| 8,781,667 B2          | 7/2014           | Wimmer et al.      | 2019/0126910 A1          | 5/2019          | Kim et al.           |                   |
| 8,783,016 B2          | 7/2014           | Gonze et al.       | 2019/0161070 A1          | 5/2019          | Kamatani et al.      |                   |
| 8,838,316 B2          | 9/2014           | Whitney et al.     | 2019/0177651 A1 *        | 6/2019          | Loper .....          | C10L 1/1641       |
| 8,883,102 B1          | 11/2014          | Lambert et al.     | 2019/0249097 A1          | 8/2019          | Cracknell et al.     |                   |
| 9,080,125 B2          | 7/2015           | Deshimaru          | 2019/0249102 A1          | 8/2019          | Martin et al.        |                   |
| 9,180,858 B2          | 11/2015          | Aoki et al.        | 2019/0263390 A1          | 8/2019          | Berger et al.        |                   |
| 9,206,379 B2          | 12/2015          | Smith              | 2019/0284496 A1          | 9/2019          | Fang                 |                   |
| 9,389,145 B2          | 7/2016           | Andreae            | 2019/0292959 A1          | 9/2019          | Dudar                |                   |
| 9,403,427 B2          | 8/2016           | Haladyna et al.    | 2019/0301329 A1          | 10/2019         | Zink et al.          |                   |
| 9,518,530 B2          | 12/2016          | Thibault et al.    | FOREIGN PATENT DOCUMENTS |                 |                      |                   |
| 9,650,034 B2          | 5/2017           | Kim                | CN                       | 103695112 B     | 6/2015               |                   |
| 9,744,966 B2          | 8/2017           | Ouchi et al.       | CN                       | 103443256 B     | 5/2016               |                   |
| 9,815,452 B2          | 11/2017          | Teraya et al.      | CN                       | 104334699 B     | 7/2017               |                   |
| 9,821,794 B2          | 11/2017          | Muta et al.        | EP                       | 2103673 B1      | 7/2015               |                   |
| 9,925,974 B2          | 3/2018           | Leone et al.       | EP                       | 2837675 B1      | 3/2017               |                   |
| 10,053,083 B2         | 8/2018           | Miyaishi           | EP                       | 2907716 A3      | 3/2017               |                   |
| 10,059,325 B2         | 8/2018           | Leone et al.       | EP                       | 2256325 A3      | 6/2017               |                   |
| 10,065,625 B2         | 9/2018           | Kawamura et al.    | EP                       | 3315590 A1      | 5/2018               |                   |
| 10,246,079 B2         | 4/2019           | Kamatani et al.    | EP                       | 2844726 B1      | 9/2019               |                   |
| 10,294,436 B2         | 5/2019           | Orlebar et al.     | EP                       | 2933320 B1 *    | 10/2019              | ..... C10M 141/10 |
| 10,392,004 B2         | 8/2019           | Iwase et al.       | EP                       | 3371280 B1      | 2/2020               |                   |
| 10,414,363 B2         | 9/2019           | Kim et al.         | GB                       | 2416601 B       | 9/2008               |                   |
| 10,435,011 B2         | 10/2019          | Gibson et al.      | IN                       | 623MUMNP2011 A  | 7/2012               |                   |
| 2007/0204594 A1       | 9/2007           | Ishii              | IN                       | 9186DELNP2014 A | 7/2015               |                   |
| 2010/0251698 A1       | 10/2010          | Hiranuma et al.    | IN                       | 201741040772 A  | 5/2019               |                   |
| 2011/0245116 A1 *     | 10/2011          | Schroeck .....     | C10M 135/10              | JP              | 5647389 B2           | 12/2014           |
|                       |                  |                    | 508/370                  | JP              | 2015059502 A *       | 3/2015            |
| 2012/0012076 A1       | 1/2012           | Atkinson et al.    | JP                       | 5819384 B2      | 11/2015              |                   |
| 2012/0138274 A1       | 6/2012           | Shin et al.        | JP                       | 5847892 B2      | 1/2016               |                   |
| 2012/0264661 A1       | 10/2012          | Tsubouchi          | JP                       | 5931250 B2      | 6/2016               |                   |
| 2012/0283162 A1       | 11/2012          | Tsubouchi          | JP                       | 2016180069 A    | 10/2016              |                   |
| 2013/0203639 A1 *     | 8/2013           | Roski .....        | C07C 309/24              | JP              | 2016194002 A         | 11/2016           |
|                       |                  |                    | 508/391                  | JP              | 2017052400 A         | 3/2017            |
| 2014/0221260 A1 *     | 8/2014           | Herz .....         | C10M 159/20              | WO              | 9406897 A1           | 3/1994            |
|                       |                  |                    | 508/175                  | WO              | 9812285 A1           | 3/1998            |
| 2015/0126419 A1       | 5/2015           | Lerasle et al.     | WO                       | 2004041960 A1   | 5/2004               |                   |
| 2015/0175925 A1 *     | 6/2015           | Dance .....        | C10M 141/08              | WO              | 2012092401 A1        | 7/2012            |
|                       |                  |                    | 508/198                  | WO              | 2015092509 A1        | 6/2015            |
| 2016/0082949 A1       | 3/2016           | Jang               | WO                       | 2018067902 A1   | 4/2018               |                   |
| 2017/0015930 A1 *     | 1/2017           | Fletcher .....     | C10M 129/50              | WO              | 2018078290 A1        | 5/2018            |
| 2017/0073607 A1       | 3/2017           | Skinner et al.     |                          | WO              | 2019036285 A1        | 2/2019            |
| 2017/0232959 A1       | 8/2017           | Bureau et al.      |                          | WO              | WO-2019094019 A1 *   | 5/2019            |
| 2017/0306254 A1       | 10/2017          | Orlebar et al.     |                          | WO              | 2019129369 A1        | 7/2019            |

\* cited by examiner

## 1

## LUBRICATING COMPOSITIONS FOR A HYBRID ENGINE

## CROSS REFERENCE TO RELATED APPLICATIONS

This application claims the benefit of U.S. provisional application No. 63/197,171, filed on Jun. 4, 2021, the entire disclosure of which is hereby incorporated by reference as if fully set forth herein.

## TECHNICAL FIELD

The disclosure relates to methods for improving catalyst life, reducing wear and friction when operating a hybrid vehicle engine. More specifically, the disclosure relates to the foregoing methods employing lubricating oil compositions comprising zinc dialkyl dithiophosphates capable of providing improved phosphorus retention and reduced wear when operating a hybrid vehicle engine.

## BACKGROUND

With the current trend toward more energy efficient vehicles, it is important to recognize that typical additives may not provide the same expected results under the operating conditions of a hybrid vehicle engine. Hybrid vehicles make use of both electrical energy stored in re-chargeable batteries and the mechanical energy converted from fuel, usually hydrocarbon based, by conventional internal combustion engines. These hybrid engines operate at temperatures of from about 70° C. to about 100° C., compared to typical internal combustion engines, which generally operate at temperatures of about 150° C.

Typical antiwear agents, for example, zinc dialkyl dithiophosphates (ZDDPs), are commonly employed in lubricating oil compositions to provide antiwear, oxidation inhibition, and/or corrosion protection. Initially, ZDDP components are reversibly absorbed onto a metal surface at low temperatures. As the temperature increases, catalytic decomposition of ZDDP to dialkyldithiophosphoryl disulfide occurs, with the disulfide absorbed onto the metal surface. From here, the thermal degradation products are formed with increasing temperature and pressure until a film is formed on the surface.

One concern that arises when employing ZDDPs in hybrid engine oil compositions is that the ZDDP does not reach the thermal degradation temperature in the low operating conditions. As a result, the ZDDP may not form a protective film surface to provide anti-wear protection. Another concern that arises is that phosphorus may volatilize, pass through the combustion chamber, and deposit on catalytic systems resulting in a loss of catalyst efficiency.

While phosphorus retention in engine oils helps improve catalytic converter life or efficiency, the benefits of phosphorus additives for wear protection also needs to be considered. Therefore, it is important to identify ZDDP components which provide a balance between these three properties under the operating conditions of hybrid vehicle engines.

## SUMMARY AND TERMS

In a first aspect, the present disclosure relates to a method for improving phosphorus retention in an internal combustion engine of a hybrid vehicle. The method includes lubri-

## 2

cating the internal combustion engine of the hybrid vehicle with a lubricating oil composition including:

greater than 50 wt. % of a base oil of lubricating viscosity; and

an amount of one or more zinc dialkyl dithiophosphate compound(s) sufficient to provide:

from about 100 ppmw phosphorus to about 1000 ppmw phosphorus, based on a total weight of the lubricating oil composition; and

from about 10 ppmw zinc to about 1200 ppmw zinc, based on the total weight of the lubricating oil composition,

wherein the one or more zinc dialkyl dithiophosphate compounds are derived from one or more primary alkyl alcohol(s), one or more secondary alkyl alcohol(s), or combinations thereof.

In the foregoing method, the phosphorus retention may be sufficient to reduce catalyst poisoning relative to a same lubricating oil composition without the one or more zinc dialkyl dithiophosphate compounds.

In each of the foregoing methods, the internal combustion engine of the hybrid vehicle may be operated at a temperature of 100° C. or less, or from about 70° C. to about 100° C.

In each of the foregoing methods, the one or more zinc dialkyl dithiophosphate compound(s) may be derived from one or more primary alkyl alcohol(s) each having an alkyl group with 3 to 8 carbon atoms.

In each of the foregoing methods, the alkyl group of the one or more primary alkyl alcohol(s) may have branching at the beta carbon relative to the hydroxyl group.

In each of the foregoing methods, the one or more zinc dialkyl dithiophosphate compound(s) is derived from one or more primary alkyl alcohol selected from the group consisting of n-propyl alcohol, isopropyl alcohol, isobutyl alcohol, n-butyl alcohol, 2-butanol, n-penyl alcohol, hexanol, methyl isobutyl carbinol, isohexanol, n-heptanol, isoheptanol, octanol, amyl alcohol, and 2-ethylhexanol.

In each of the foregoing methods, the one or more zinc dialkyl dithiophosphate compound(s) may be derived from two or more primary alkyl alcohols.

In each of the foregoing methods, the one or more zinc dialkyl dithiophosphate compound(s) may be derived the one or more secondary alkyl alcohol(s) having an alkyl group with 3 to 8 carbon atoms.

In each of the foregoing methods, the one or more zinc dialkyl dithiophosphate compound(s) may be derived from a secondary alkyl alcohol selected from the group consisting of isopropyl alcohol, amyl alcohol, and methyl isobutyl carbinol.

In each of the foregoing methods, the one or more zinc dialkyl dithiophosphate compound(s) may be derived from two or more secondary alkyl alcohols.

In each of the foregoing methods, the one or more zinc dialkyl dithiophosphate compound(s) may be derived from a molar ratio of the one or more primary alkyl alcohol(s) to the one or more secondary alkyl alcohol(s) of from 100:20 to 50:50.

In each of the foregoing methods, the one or more zinc dialkyl dithiophosphate compound(s) may be a zinc to phosphorus molar ratio of from 1.08 to 1.3.

In each of the foregoing methods, wherein the one or more zinc dialkyl dithiophosphate compound(s) may comprise an average number of total carbon atoms per mole of phosphorus of from about 5 to about 30, or from about 8 to about 20.

In each of the foregoing methods, the lubricating oil composition may further comprise a calcium-sulfonate detergent. The calcium-sulfonate detergent may comprise an overbased calcium-sulfonate detergent and/or a low-based/neutral calcium-sulfonate detergent. The lubricating oil composition may comprise from about 500 ppmw to about 2000 ppmw calcium from the calcium-sulfonate detergent, based on a total weight of the lubricating oil composition.

In each of the foregoing methods, the lubricating oil composition may comprise a borated succinimide dispersant.

In each of the foregoing methods, the lubricating oil composition may further comprise a succinimide dispersant. In some embodiments, the succinimide dispersant is a borated succinimide. Preferably, the borated succinimide is present in an amount of from about 5 ppmw to about 300 ppmw.

In each of the foregoing methods, the lubricating oil composition may further comprise one or more components selected from the group consisting of organic friction modifier(s), molybdenum-containing compound(s), calcium sulfonate detergent(s), antioxidant(s), antifoam agent(s), pour point depressant(s), and viscosity index improver(s).

In a second aspect, the disclosure relates to a method for reducing wear in an internal combustion engine of a hybrid vehicle comprising lubricating the internal combustion engine of the hybrid vehicle with a lubricating oil composition comprising:

greater than 50 wt. % of a base oil of lubricating viscosity; and

an amount of one or more zinc dialkyl dithiophosphate compound(s) sufficient to provide:

from about 100 ppmw phosphorus to about 1000 ppmw phosphorus, based on a total weight of the lubricating oil composition, and

from about 10 ppmw zinc to about 1200 ppmw zinc, based on the total weight of the lubricating oil composition.

In the second embodiment, the one or more zinc dialkyl dithiophosphate compounds may be derived from 100 mole % of one or more primary alkyl alcohol(s).

In each of the foregoing second embodiments, the one or more zinc dialkyl dithiophosphate compound(s) may have a zinc to phosphorus molar ratio of from 1.20 and greater, or from about 1.20 to about 5, or from about 1.27 and greater.

In each of the foregoing second embodiments, the internal combustion engine of the hybrid vehicle may be operated at a temperature of 100° C. or less.

In each of the foregoing second embodiments, the one or more zinc dialkyl dithiophosphate compound(s) may be derived from the one or more primary alkyl alcohol(s) having an alkyl group with 3 to 9 carbon atoms.

In each of the foregoing second embodiments, the one or more zinc dialkyl dithiophosphate compound(s) may comprise an average number of total carbon atoms per mole of phosphorus of from about 8 to about 30, or from about 12 to about 20.

In each of the foregoing second embodiments, the alkyl group of the one or more primary alkyl alcohol(s) may have branching at the beta carbon relative to the hydroxyl group. In each of the foregoing second embodiments, the one or more zinc dialkyl dithiophosphate compound(s) may be derived from one or more primary alkyl alcohol(s) selected from the group consisting of n-propyl alcohol, isopropyl alcohol, n-butyl alcohol, 2-butanol, n-penyl alcohol, hexa-

nol, methyl isobutyl carbinol, isohexanol, n-heptanol, isoheptanol, octanol, isobutyl alcohol, amyl alcohol, and 2-ethylhexanol.

In each of the foregoing second embodiments, the one or more zinc dialkyl dithiophosphate compound(s) may be derived from two or more primary alkyl alcohols.

In each of the foregoing second embodiments, the one or more zinc dialkyl dithiophosphate compound(s) may be overbased with zinc oxide.

10 In each of the foregoing second embodiments, the lubricating oil composition may further comprise a calcium-sulfonate detergent. The calcium-sulfonate detergent may comprise an overbased calcium-sulfonate detergent and/or a low-based/neutral calcium-sulfonate detergent. The lubricating oil composition may comprise from about 500 ppmw to about 2000 ppmw calcium from the calcium-sulfonate detergent, based on a total weight of the lubricating oil composition.

20 In each of the foregoing second embodiments, the lubricating oil composition may further comprise a succinimide dispersant. In some embodiments, the succinimide dispersant is a borated succinimide dispersant. In some embodiments, the lubricating oil composition comprises about 5 ppmw of boron to about 300 ppmw of boron from the borated succinimide dispersant.

25 In each of the foregoing second embodiments, the lubricating oil composition may further comprise one or more components selected from the group consisting of organic friction modifier(s), molybdenum-containing compound(s) calcium sulfonate detergent(s), antioxidant(s), antifoam agent(s), pour point depressant(s), and viscosity index improver(s).

30 In a third aspect, the disclosure relates to a lubricating oil composition for use in an internal combustion engine of a hybrid vehicle, comprising:

greater than 50 wt. % of a base oil of lubricating viscosity; and

an amount of one or more zinc dialkyl dithiophosphate compound(s) sufficient to provide:

from about 100 ppmw phosphorus to about 1000 ppmw phosphorus, based on a total weight of the lubricating oil composition, and

from about 10 ppmw zinc to about 1200 ppmw zinc, based on the total weight of the lubricating oil composition.

35 In the third embodiment, the one or more zinc dialkyl dithiophosphate compounds may be derived from one or more primary alkyl alcohol(s), one or more secondary alkyl alcohol(s), or combinations thereof and wherein the one or more zinc dialkyl dithiophosphate compound(s) is derived from a molar ratio of the one or more primary alkyl alcohol(s) to the one or more secondary alkyl alcohol(s) of from 100:20 to 50:50. The one or more zinc dialkyl dithiophosphate compound(s) may have a zinc to phosphorus molar ratio of from 1.08 to 1.3.

40 In each of the foregoing third embodiments, the lubricating oil composition may be configured for use in an internal combustion engine of the hybrid vehicle that is operated at a temperature of 100° C. or less.

45 In each of the foregoing third embodiments, the lubricating oil composition may further comprise a calcium-sulfonate detergent. The calcium-sulfonate detergent may comprise an overbased calcium-sulfonate detergent and/or a low-based/neutral calcium-sulfonate detergent. The lubricating oil composition may comprise from about 500 ppmw to

about 2000 ppmw calcium from the calcium-sulfonate detergent, based on a total weight of the lubricating oil composition.

In each of the foregoing third embodiments, the lubricating oil composition may further comprise a succinimide dispersant. In some embodiments, the succinimide dispersant is a borated succinimide dispersant. In some embodiments, the lubricating oil composition comprises about 5 ppmw of boron to about 300 ppmw of boron from the borated succinimide dispersant.

In each of the foregoing third embodiments, the lubricating oil composition may further comprise one or more components selected from the group consisting of organic friction modifier(s), molybdenum-containing compound(s) calcium sulfonate detergent(s), antioxidant(s), antifoam agent(s), pour point depressant(s), and viscosity index improver(s).

The following definitions of terms are provided in order to clarify the meanings of certain terms as used herein.

The terms "oil composition," "lubrication composition," "lubricating oil composition," "lubricating oil," "lubricant composition," "lubricating composition," "fully formulated lubricant composition," "lubricant," "crankcase oil," "crankcase lubricant," "engine oil," "engine lubricant," "motor oil," and "motor lubricant" are considered synonymous, fully interchangeable terminology referring to the finished lubrication product comprising a major amount of a base oil plus a minor amount of an additive composition.

As used herein, the terms "additive package," "additive concentrate," "additive composition," "engine oil additive package," "engine oil additive concentrate," "crankcase additive package," "crankcase additive concentrate," "motor oil additive package," "motor oil concentrate," are considered synonymous, fully interchangeable terminology referring to the portion of the lubricating oil composition excluding the major amount of base oil stock mixture. The additive package may or may not include the viscosity index improver or pour point depressant.

The term "overbased" relates to metal salts, such as metal salts of sulfonates, carboxylates, salicylates, and/or phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or superbased salts and may be salts of organic sulfur acids, carboxylic acids, salicylates, and/or phenols.

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having a predominantly hydrocarbon character. Each hydrocarbyl group is independently selected from hydrocarbon substituents, and substituted hydrocarbon substituents containing one or more of halo groups, hydroxyl groups, alkoxy groups, mercapto groups, nitro groups, nitroso groups, amino groups, pyridyl groups, furyl groups, imidazolyl groups, oxygen and nitro-

gen, and wherein no more than two non-hydrocarbon substituents are present for every ten carbon atoms in the hydrocarbyl group.

As used herein, the term "hydrocarbylene substituent" or "hydrocarbylene group" is used in its ordinary sense, which is well-known to those skilled in the art. Specifically, it refers to a group that is directly attached at two locations of the molecule to the remainder of the molecule by a carbon atom and having predominantly hydrocarbon character.

- 10 Each hydrocarbylene group is independently selected from divalent hydrocarbon substituents, and substituted divalent hydrocarbon substituents containing halo groups, alkyl groups, aryl groups, alkylaryl groups, arylalkyl groups, hydroxyl groups, alkoxy groups, mercapto groups, nitro groups, nitroso groups, amino groups, pyridyl groups, furyl groups, imidazolyl groups, oxygen and nitrogen, and wherein no more than two non-hydrocarbon substituents is present for every ten carbon atoms in the hydrocarbylene group.

- 20 As used herein, the term "percent by weight", unless expressly stated otherwise, means the percentage the recited component represents to the weight of the entire composition.

- 25 The terms "soluble," "oil-soluble," or "dispersible" used herein may, but does not necessarily, indicate that the compounds or additives are soluble, dissolvable, miscible, or capable of being suspended in the oil in all proportions. The foregoing terms do mean, however, that they are, for instance, soluble, suspendable, dissolvable, or stably dispersible in oil to an extent sufficient to exert their intended effect in the environment in which the oil is employed. Moreover, the additional incorporation of other additives may also permit incorporation of higher levels of a particular additive, if desired.

- 30 The term "TBN" as employed herein is used to denote the Total Base Number in mg KOH/g as measured by the method of ASTM D2896 or ASTM D4739 or DIN 51639-1.

- 35 The term "alkyl" as employed herein refers to straight, branched, cyclic, and/or substituted saturated chain moieties of from about 1 to about 100 carbon atoms.

- 40 The term "alkenyl" as employed herein refers to straight, branched, cyclic, and/or substituted unsaturated chain moieties of from about 3 to about 10 carbon atoms.

- 45 The term "aryl" as employed herein refers to single and multi-ring aromatic compounds that may include alkyl, alkenyl, alkylaryl, amino, hydroxyl, alkoxy, halo substituents, and/or heteroatoms including, but not limited to, nitrogen, oxygen, and sulfur.

- 50 Lubricants, combinations of components, or individual components of the present description may be suitable for use in hybrid vehicles. Hybrid vehicles include various types of internal combustion engines which are used in combination with an electrical or battery source of power. The engines of hybrid vehicles typically operate at a temperature of less than 100° C., compared to typical internal combustion engines which operate at around 150° C. Suitable engine types may include, but are not limited to heavy duty diesel, passenger car, or light duty diesel. The internal combustion engine may be a diesel fueled engine, a gasoline fueled engine, a natural gas fueled engine, a bio-fueled engine, a mixed diesel/biofuel fueled engine, a mixed gasoline/biofuel fueled engine, an alcohol fueled engine, a mixed gasoline/alcohol fueled engine, a compressed natural gas (CNG) fueled engine, or mixtures thereof. A diesel engine may be a compression ignited engine. A gasoline engine may be a spark-ignited engine. The internal combustion engine may be a 2-stroke, 4-stroke, or rotary engine. Suitable

internal combustion engines include aviation piston engines, low-load diesel engines, and motorcycle, automobile, and truck engines.

The internal combustion engine may contain components of one or more of an aluminum-alloy, lead, tin, copper, cast iron, magnesium, ceramics, stainless steel, composites, and/or mixtures thereof. The components may be coated, for example, with a diamond-like carbon coating, a lubrified coating, a phosphorus-containing coating, molybdenum-containing coating, a graphite coating, a nano-particle-containing coating, and/or mixtures thereof. The aluminum-alloy may include aluminum silicates, aluminum oxides, or other ceramic materials. In one embodiment the aluminum-alloy is an aluminum-silicate surface. As used herein, the term "aluminum alloy" is intended to be synonymous with "aluminum composite" and to describe a component or surface comprising aluminum and another component intermixed or reacted on a microscopic or nearly microscopic level, regardless of the detailed structure thereof. This would include any conventional alloys with metals other than aluminum as well as composite or alloy-like structures with non-metallic elements or compounds such with ceramic-like materials.

The lubricating oil composition for an internal combustion engine may be suitable for any engine lubricant irrespective of the sulfur, phosphorus, or sulfated ash (ASTM D-874) content. The sulfur content of the engine oil lubricant may be about 1 wt. % or less, or about 0.8 wt. % or less, or about 0.5 wt. % or less, or about 0.3 wt. % or less, or about 0.2 wt. % or less. In one embodiment the sulfur content may be in the range of about 0.001 wt. % to about 0.5 wt. %, or about 0.01 wt. % to about 0.3 wt. %. The phosphorus content may be about 0.2 wt. % or less, or about 0.1 wt. % or less, or about 0.085 wt. % or less, or about 0.08 wt. % or less, or even about 0.06 wt. % or less, about 0.055 wt. % or less, or about 0.05 wt. % or less. In one embodiment the phosphorus content may be about 50 ppm to about 1000 ppm, or about 325 ppm to about 850 ppm. The total sulfated ash content may be about 2 wt. % or less, or about 1.5 wt. % or less, or about 1.1 wt. % or less, or about 1 wt. % or less, or about 0.8 wt. % or less, or about 0.5 wt. % or less. In one embodiment the sulfated ash content may be about 0.05 wt. % to about 0.9 wt. %, or about 0.1 wt. % or about 0.2 wt. % to about 0.45 wt. %. In another embodiment, the sulfur content may be about 0.4 wt. % or less, the phosphorus content may be about 0.08 wt. % or less, and the sulfated ash is about 1 wt. % or less. In yet another embodiment the sulfur content may be about 0.3 wt. % or less, the phosphorus content is about 0.05 wt. % or less, and the sulfated ash may be about 0.8 wt. % or less.

In one embodiment the lubricating oil composition is an engine oil, wherein the lubricating oil composition may have (i) a sulfur content of about 0.5 wt. % or less, (ii) a phosphorus content of about 0.1 wt. % or less, and (iii) a sulfated ash content of about 1.5 wt. % or less.

In some embodiments, the lubricating oil composition is suitable for use with engines powered by low sulfur fuels, such as fuels containing about 1 to about 5% sulfur. Highway vehicle fuels contain about 15 ppm sulfur (or about 0.0015% sulfur).

Low speed diesel typically refers to marine engines, medium speed diesel typically refers to locomotives, and high speed diesel typically refers to highway vehicles. The lubricating oil composition may be suitable for only one of these types or all.

Further, lubricants of the present description may be suitable to meet one or more industry specification require-

ments such as IL-SAC GF-3, GF-4, GF-5, GF-6, PC-11, CF, CF-4, CH-4, CK-4, FA-4, CJ-4, CI-4 Plus, CI-4, API SG, SJ, SL, SM, SN, ACEA Al/B1, A2/B2, A3/B3, A3/B4, A5/B5, A7/B7 C1, C2, C3, C4, C5, C6, E4/E6/E7/E9, Euro 5/6, 5 JASO DL-1, Low SAPS, Mid SAPS, or original equipment manufacturer specifications such as Dexos<sup>TM</sup> 1, Dexos<sup>TM</sup> 2, MB-Approval 229.1, 229.3, 229.5, 229.51/229.31, 229.52, 229.6, 229.71, 226.5, 226.51, 228.0/1, 228.2/3, 228.31, 228.5, 228.51, 228.61, VW 501.01, 502.00, 503.00/503.01, 10 504.00, 505.00, 505.01, 506.00/506.01, 507.00, 508.00, 509.00, 508.88, 509.99, BMW Longlife-01, Longlife-01 FE, Longlife-04, Longlife-12 FE, Longlife-14 FE+, Longlife-17 FE+, Porsche A40, C30, Peugeot Citroën Automobiles B71 2290, B71 2294, B71 2295, B71 2296, B71 2297, B71 2300, 15 B71 2302, B71 2312, B71 2007, B71 2008, Renault RN0700, RN0710, RN0720, Ford WSS-M2C153-H, WSS-M2C930-A, WSS-M2C945-A, WSS-M2C913A, WSS-M2C913-B, WSS-M2C913-C, WSS-M2C913-D, WSS-M2C948-B, WSS-M2C948-A, GM 6094-M, Chrysler 20 MS-6395, Fiat 9.55535 G1, G2, M2, N1, N2, Z2, Si, S2, S3, S4, T2, DS1, DSX, GH2, GS1, GSX, CR1, Jaguar Land Rover STJLR.03.5003, STJLR.03.5004, STJLR.03.5005, STJLR.03.5006, STJLR.03.5007, STJLR.51.5122 or any 25 past or future PCMO or HDD specifications not mentioned herein. In some embodiments for passenger car motor oil (PCMO) applications, the amount of phosphorus in the finished fluid is 1000 ppm or less or 900 ppm or less or 800 ppm or less.

Other hardware may not be suitable for use with the 30 disclosed lubricant. A "functional fluid" is a term which encompasses a variety of fluids including but not limited to tractor hydraulic fluids, power transmission fluids including automatic transmission fluids, continuously variable transmission fluids and manual transmission fluids, hydraulic fluids, including tractor hydraulic fluids, some gear oils, power steering fluids, fluids used in wind turbines, compressors, some industrial fluids, and fluids related to power train components. It should be noted that within each of 35 these fluids such as, for example, automatic transmission fluids, there are a variety of different types of fluids due to the various transmissions having different designs which have led to the need for fluids of markedly different functional characteristics. This is contrasted by the term "lubricating fluid" which is not used to generate or transfer power.

40 With respect to tractor hydraulic fluids, for example, these fluids are all-purpose products used for all lubricant applications in a tractor except for lubricating the engine. These lubricating applications may include lubrication of gearboxes, power take-off and clutch(es), rear axles, reduction gears, wet brakes, and hydraulic accessories.

50 When the functional fluid is an automatic transmission fluid, the automatic transmission fluids must have enough friction for the clutch plates to transfer power. However, the friction coefficient of fluids has a tendency to decline due to 55 the temperature effects as the fluid heats up during operation. It is important that the tractor hydraulic fluid or automatic transmission fluid maintain its high friction coefficient at elevated temperatures, otherwise brake systems or automatic transmissions may fail. This is not a function of an engine oil.

Tractor fluids, and for example Super Tractor Universal Oils (STUOs) or Universal Tractor Transmission Oils (UTTOs), may combine the performance of engine oils with 60 transmissions, differentials, final-drive planetary gears, wet-brakes, and hydraulic performance. While many of the additives used to formulate a UTTO or a STUO fluid are similar in functionality, they may have deleterious effect if

not incorporated properly. For example, some anti-wear and extreme pressure additives used in engine oils can be extremely corrosive to the copper components in hydraulic pumps. Detergents and dispersants used for gasoline or diesel engine performance may be detrimental to wet brake performance. Friction modifiers specific to quiet wet brake noise, may lack the thermal stability required for engine oil performance. Each of these fluids, whether functional, tractor, or lubricating, are designed to meet specific and stringent manufacturer requirements.

The present disclosure provides novel lubricating oil blends formulated for use as automotive crankcase lubricants. The present disclosure provides novel lubricating oil blends formulated for use as 2T and/or 4T motorcycle crankcase lubricants. Embodiments of the present disclosure may provide lubricating oils suitable for crankcase applications and having improvements in the following characteristics: air entrainment, alcohol fuel compatibility, antioxidant, antiwear performance, biofuel compatibility, foam reducing properties, friction reduction, fuel economy, pre-ignition prevention, rust inhibition, sludge and/or soot dispersability, piston cleanliness, deposit formation, and water tolerance.

Engine oils of the present disclosure may be formulated by the addition of one or more additives, as described in detail below, to an appropriate base oil formulation. The additives may be combined with a base oil in the form of an additive package (or concentrate) or, alternatively, may be combined individually with a base oil (or a mixture of both). The fully formulated engine oil may exhibit improved performance properties, based on the additives added and their respective proportions.

Additional details and advantages of the disclosure will be set forth in part in the description which follows, and/or may be learned by practice of the disclosure. The details and advantages of the disclosure may be realized and attained by means of the elements and combinations particularly pointed out in the appended claims. It is to be understood that both the foregoing general description and the following detailed description are exemplary and explanatory only and are not restrictive of the disclosure, as claimed.

#### DETAILED DESCRIPTION

The invention relates to methods for improving phosphorus retention in an internal combustion engine of a hybrid vehicle by lubricating the internal combustion engine of the hybrid vehicle with a lubricating oil composition, where the phosphorus retention is sufficient to reduce catalyst poisoning relative to a same lubricating oil composition without the one or more zinc dialkyl dithiophosphate compounds.

In another aspect, the invention relates to methods for reducing wear in an internal combustion engine of a hybrid vehicle including lubricating the internal combustion engine of the hybrid vehicle with a lubricating oil composition.

The lubricating oil compositions employed in the foregoing methods includes greater than 50 wt. % of a base oil, based on a total weight of the lubricating oil composition, and one or more zinc dialkyl dithiophosphate compounds, wherein the one or more zinc dialkyl dithiophosphate compound(s) are derived from a molar ratio of primary alkyl alcohol to secondary alkyl alcohol of from about 100:0 to 0:100.

#### Zinc Dialkyl Dithiophosphate Compound(s)

The lubricating oil composition of the disclosure for use in the methods for improving phosphorus retention and improving wear properties in an internal combustion engine

of a hybrid vehicle contains an amount of one or more zinc dialkyl dithiophosphates (ZDDP).

The ZDDP is present in the lubricating oil composition in amounts of from about 0.01 wt. % to about 15 wt. %, or about 0.01 wt. % to about 10 wt. %, or about 0.05 wt. % to about 5 wt. %, or about 0.1 wt. % to about 3 wt. % based on the total weight of the lubricating oil composition.

The ZDDP compounds can comprise ZDDPs derived from primary alkyl alcohols, secondary alkyl alcohols, or a combination of primary and secondary alkyl alcohols. The primary alkyl alcohols and secondary alkyl alcohols used to prepare the ZDDP agent may have an alkyl group including 1 to 20 carbon atoms, or from about 1 to 18 carbon atoms, or from about 1 to about 16 carbon atoms, or 2 to 12 carbon atoms, or about 3 to about 8 carbon atoms. Preferably, the primary alkyl alcohols have branching at the beta carbon relative to the hydroxyl group.

For example, an alcohol with branching at the beta ( $\beta$ ) carbon, would be branching at the second carbon counted from the oxygen atom of the hydroxyl group.



Suitable examples of primary alkyl alcohols and secondary alkyl alcohols for use in preparing the ZDDP agent may be selected from the group consisting of n-propyl alcohol, isopropyl alcohol, n-butyl alcohol, 2-butanol, isobutyl alcohol, n-pentyl alcohol, amyl alcohol, hexanol, methyl isobutyl carbinol, isohexanol, n-heptanol, isoheptanol, octanol, nonanol, decanol, undecanol, dodecanol, tridecanol, tetradecanol, pentadecanol, hexadecanol, heptadecanol, octadecanol, nonadecanol, eicosanol, and 2-ethylhexanol.

The molar ratio of primary alkyl alcohol to secondary alkyl alcohol used to make the ZDDPs in the lubricating oil composition is from about 100:0 to 0:100, or from about 100:0 to 50:50, or from 100:0 to 60:40. The ZDDP's may have a P:Zn molar ratio of from about 1.08 to 1.3, or from about 1.08 to 1.2, or from about 1.09 to about 1.15. In some embodiments, the one or more zinc dialkyl dithiophosphate compound(s) may be overbased with zinc oxide.

In some embodiments, the additive composition comprises at least two different zinc dialkyl dithiophosphate compound(s). The two alkyl groups on the zinc dialkyl dithiophosphate compound(s) may be the same or different.

In some embodiments, 100 mole percent of the alkyl groups of the one or more zinc dialkyl dithiophosphate compound(s) may be derived from one or more primary alcohol groups. In some embodiments, 100 mole percent of the alkyl groups of the one or more zinc dialkyl dithiophosphate compound(s) may be derived from one or more secondary alcohol groups. In some embodiments, mixtures of all primary alcohol zinc dialkyl dithiophosphate salts and all secondary alcohol zinc dialkyl dithiophosphate salts are provided.

The alcohols suitable for producing the zinc dialkyl dithiophosphate salts may be primary alkyl alcohols, secondary alkyl alcohols, or a mixture of primary and secondary alcohols. In an embodiment, the additive package comprises one zinc dialkyl dithiophosphate salt derived from an alcohol comprising a primary alkyl group and another zinc dialkyl dithiophosphate salt derived from an alcohol comprising a secondary alkyl group. In another embodiment, the zinc dialkyl dithiophosphate compound is derived from at least two secondary alcohols. The alcohols may contain any of branched, cyclic, or straight chains.

The one or more zinc dialkyl dithiophosphate salt may be oil soluble salts of dihydrocarbyl dithiophosphoric acids and may be represented by the following formula:



wherein  $R_5$  and  $R_6$  may be the same or different alkyl groups containing from 1 to 20 carbon atoms, or from about 1 to 18 carbon atoms, or from about 1 to about 16 carbon atoms, or 2 to 12 carbon atoms, or about 3 to about 8 carbon atoms, and including moieties such as alkyl, and cycloalkyl moieties. Thus, the moieties may, for example, be ethyl, n-propyl, i-propyl, n-butyl, butyl, sec-butyl, amyl, n-hexyl, i-hexyl, n-octyl, decyl, dodecyl, undecyl, dodecyl, tridecyl, tetradecyl, pentadecyl, hexadecyl, heptadecyl, octadecyl, nonadecyl, eicosyl, 2-ethylhexyl, cyclohexyl, or methylcyclopentyl.

The average number of total number of carbon atoms per mole of phosphorus for a ZDDP compound may be calculated by dividing by two the sum of the carbon atoms in the four alkyl groups  $R_5$  and  $R_6$  provided to the ZDDP compound by alcohol(s) used to make the ZDDP compound. For example, for a single ZDDP compound, if  $R_5$  is a  $C_3$ -alkyl group and  $R_6$  is a  $C_6$  alkyl group, the total number of carbon atoms is  $3+3+6+6=18$ . Dividing this by two moles of phosphorus per mole of ZDDP gives an average total number of carbon atoms per mole of phosphorus of 9.

The average total number of carbon atoms per mole of phosphorus (ATCP) for compositions containing one or more ZDDP compounds may be calculated from the alcohol (s) used to make the ZDDP compounds according to the following formula:

$$ATCP = 2 * [(\text{mol\% of } alc1 * \# \text{ of } C \text{ atoms in } alc1) + (\text{mol\% of } alc2 * \# \text{ of } C \text{ atoms in } alc2) + (\text{mol\% of } alc3 * \# \text{ of } C \text{ atoms in } alc3) + \dots \text{ etc.}]$$

wherein alc1, alc2 and alc3 each represent a different alcohol used to make the ZDDP compound(s) and the mol % is the molar percentage of each of the alcohols that was present in the reaction mixture used to make the ZDDP compound(s). The "etc." indicates that if more than three alcohols are used to make the ZDDP compound(s), the formula can be expanded to include each of the alcohols present in the reaction mixture.

The average total number of carbon atoms from both  $R_5$  and  $R_6$  in the ZDDP is greater than 2 carbon atoms per mole of phosphorus, and in one embodiment in the range from greater than 4 to 40 carbon atoms, or from greater than 5 to about 30 carbon atoms, and in one embodiment in the range from greater than 6 to about 16 carbon atoms, and in one embodiment in the range from about 6 to about 15 carbon atoms, and in one embodiment in the range from about 9 to about 15 carbon atoms, and in one embodiment about 12 carbon atoms per mole of phosphorus.

The dialkyl dithiophosphate zinc salts may be prepared in accordance with known techniques by first forming a dialkyl dithiophosphoric acid (DDPA), usually by reaction of one or more alcohols and then neutralizing the formed DDPA with a zinc compound. To make the zinc salt, any basic or neutral zinc compound could be used but the oxides, hydroxides, and carbonates are most generally employed. The zinc

dialkyl dithiophosphates of component (i) may be made by a process such as the process generally described in U.S. Pat. No. 7,368,596.

In some embodiments, the at least one zinc dialkyl dithiophosphate salt may be present in the lubricating oil in an amount sufficient to provide from about 100 to about 1000 ppm phosphorus, or from about 200 to about 1000 ppm phosphorus, or from about 300 to about 900 ppm phosphorus, or from about 400 to about 800 ppm phosphorus, or from about 550 to about 700 ppm phosphorus, based on the total weight of the lubricating oil composition.

In some embodiments, the at least one zinc dialkyl dithiophosphate salt may be present in the lubricating oil in an amount sufficient to provide from about 10 ppmw zinc to about 1200 ppmw zinc, or from about 100 ppmw zinc to about 1100 ppmw zinc, or from about 200 ppmw zinc to about 1000 ppmw zinc, based on the total weight of the lubricating oil composition.

The use of one or more ZDDP compounds derived from

20 100% of one or more primary alkyl alcohols with a ratio of Zn to P of 1.270 and greater unexpectedly provides improved phosphorus retention across a wide variety of ZDDP compounds when operating at temperatures of about 100° C. or less relative to the same lubricating oil compo-

25 sitions except lacking ZDDP compounds. Specifically, to improve phosphorus retention the use of one or more ZDDP compounds derived from 100 mole percent of one or more primary alkyl alcohols, or 100 mole percent of one or more secondary alkyl alcohols, or a molar ratio of one or more

30 primary alkyl alcohols to one or more secondary alkyl alcohols of from 100:20 to 50:50, or about 60:40, unexpectedly provided increased phosphorus retention when operating at temperatures about 100° C. or less. In some embodiments, the method for improving phosphorus retention

35 comprising lubricating the internal combustion engine of a hybrid vehicle with one or more zinc dialkyl dithiophosphate compounds (s) comprising an average number of total carbon atoms per mole of phosphorus of from about 5 to about 30, or from about 8 to 20.

40 The use of one or more ZDDP compounds derived from  
100 mole percent of one or more primary alkyl alcohol(s)  
with a molar ratio of Zn to P from the one or more ZDDP  
compounds of 1.270 and greater unexpectedly provides  
improved wear results when operating at temperatures about  
45 100° C. or less or about 70° C., relative to lubricating oil  
compositions comprising ZDDP compounds derived from a  
mixture of primary and secondary alkyl alcohols or a Zn to  
P molar ratio of less than 1.270. Specifically, to reduce wear,  
the use of one or more ZDDP compounds derived from 100  
50 mole percent of one or more primary alkyl alcohols and a  
molar ratio of Zn to P from the one or more ZDDP  
compounds of 1.270 and greater unexpectedly provides  
reduced wear results when operating at temperatures about  
100° C. or less. In some embodiments, the method for  
55 reducing wear comprises lubricating the internal combustion  
engine of a hybrid vehicle with one or more zinc dialkyl  
dithiophosphate compounds (s) comprising an average num-  
ber of total carbon atoms per mole of phosphorus of from  
about 8 to about 30, or from about 12 to about 20.

60 The present invention can include overbased ZDDP's which are basic ZDDP's. The term basic ZDDP's or equivalent expressions, is used herein to describe those zinc salts wherein the metal substituent is present in stoichiometrically greater amounts than the phosphorus acid radical. For 65 instance, normal or neutral zinc phosphorodithioate has two equivalents (i.e., 1 mole) of zinc per two equivalents (i.e., 2 moles) of a phosphorodithioic acid, whereas a basic zinc

diorganophosphorodithioate has more than two equivalents of zinc per two equivalents of the phosphorodithioic acid.

For instance, the overbasing can be performed with a basic zinc compound such as zinc oxide. The amount of basic zinc compound required to give the desired overbasing is not critical. The essential factor is that there be present in the reaction mixture sufficient zinc compound for the overbasing reaction. Although it is not absolutely essential, it has been found that the reaction proceeds in a more satisfactory way if a slight excess of zinc compound over the amount required for reaction is used. This excess should be kept at a minimum level to the necessity for removing large amounts of solid from the final product. As a general statement, the excess of zinc compound should not exceed 10-15 percent by weight.

#### Base Oil

The base oil used in the lubricating oil compositions herein may be selected from any of the base oils in Groups I-V as specified in the American Petroleum Institute (API) Base Oil Interchangeability Guidelines. The five base oil groups are as follows:

| Base oil Category | Sulfur (%)                                          | Saturates (%) | Viscosity Index |
|-------------------|-----------------------------------------------------|---------------|-----------------|
| Group I           | >0.03                                               | and/or        | <90             |
| Group II          | ≤0.03                                               | and           | ≥90             |
| Group III         | ≤0.03                                               | and           | ≥90             |
| Group IV          | All polyalphaolefins (PAOs)                         |               | ≥120            |
| Group V           | All others not included in Groups I, II, III, or IV |               |                 |

Groups I, II, and III are mineral oil process stocks. Group IV base oils contain true synthetic molecular species, which are produced by polymerization of olefinically unsaturated hydrocarbons. Many Group V base oils are also true synthetic products and may include diesters, polyol esters, polyalkylene glycols, alkylated aromatics, polyphosphate esters, polyvinyl ethers, and/or polyphenyl ethers, and the like, but may also be naturally occurring oils, such as vegetable oils. It should be noted that although Group III base oils are derived from mineral oil, the rigorous processing that these fluids undergo causes their physical properties to be very similar to some true synthetics, such as PAOs. Therefore, oils derived from Group III base oils may be referred to as synthetic fluids in the industry. Group II+ may comprise high viscosity index Group II.

The base oil used in the disclosed lubricating oil composition may be a mineral oil, animal oil, vegetable oil, synthetic oil, synthetic oil blends, or mixtures thereof. Suitable oils may be derived from hydrocracking, hydrogenation, hydrofinishing, unrefined, refined, and re-refined oils, and mixtures thereof.

Unrefined oils are those derived from a natural, mineral, or synthetic source without or with little further purification treatment. Refined oils are similar to the unrefined oils except that they have been treated in one or more purification steps, which may result in the improvement of one or more properties. Examples of suitable purification techniques are solvent extraction, secondary distillation, acid or base extraction, filtration, percolation, and the like. Oils refined to the quality of an edible may or may not be useful.

Edible oils may also be called white oils. In some embodiments, lubricating oil compositions are free of edible or white oils.

Re-refined oils are also known as reclaimed or reprocessed oils. These oils are obtained similarly to refined oils using the same or similar processes. Often these oils are additionally processed by techniques directed to removal of spent additives and oil breakdown products.

Mineral oils may include oils obtained by drilling or from plants and animals or any mixtures thereof. For example, such oils may include, but are not limited to, castor oil, lard oil, olive oil, peanut oil, corn oil, soybean oil, and linseed oil, as well as mineral lubricating oils, such as liquid petroleum oils and solvent-treated or acid-treated mineral lubricating oils of the paraffinic, naphthenic or mixed paraffinic-naphthenic types. Such oils may be partially or fully hydrogenated, if desired. Oils derived from coal or shale may also be useful.

Useful synthetic lubricating oils may include hydrocarbon oils such as polymerized, oligomerized, or interpolymerized olefins (e.g., polybutylenes, polypropylenes, propyleneisobutylene copolymers); poly(1-hexenes), poly(1-octenes), trimers or oligomers of 1-decene, e.g., poly(1-decenes), such materials being often referred to as a-olefins, and mixtures thereof; alkyl-benzenes (e.g. dodecylbenzenes, tetradecylbenzenes, dinonylbenzenes, di-(2-ethylhexyl)-benzenes); polyphenyls (e.g., biphenyls, terphenyls, alkylated polyphenyls); diphenyl alkanes, alkylated diphenyl alkanes, alkylated diphenyl ethers and alkylated diphenyl sulfides and the derivatives, analogs and homologs thereof or mixtures thereof. Polyalphaolefins are typically hydrogenated materials.

Other synthetic lubricating oils include polyol esters, diesters, liquid esters of phosphorus-containing acids (e.g., tricresyl phosphate, trioctyl phosphate, and the diethyl ester of decane phosphonic acid), or polymeric tetrahydrofurans. Synthetic oils may be produced by Fischer-Tropsch reactions and typically may be hydroisomerized Fischer-Tropsch hydrocarbons or waxes. In one embodiment oils may be prepared by a Fischer-Tropsch gas-to-liquid synthetic procedure as well as other gas-to-liquid oils.

The major amount of base oil included in a lubricating composition may be selected from the group consisting of Group I, Group II, a Group III, a Group IV, a Group V, and a combination of two or more of the foregoing, and wherein the major amount of base oil is other than base oils that arise from provision of additive components or viscosity index improvers in the composition. In another embodiment, the major amount of base oil included in a lubricating composition may be selected from the group consisting of Group II, a Group III, a Group IV, a Group V, and a combination of two or more of the foregoing, and wherein the major amount of base oil is other than base oils that arise from provision of additive components or viscosity index improvers in the composition.

The amount of the oil of lubricating viscosity present may be the balance remaining after subtracting from 100 wt. % the sum of the amount of the performance additives inclusive of viscosity index improver(s) and/or pour point depressant(s) and/or other top treat additives. For example, the oil of lubricating viscosity that may be present in a finished fluid may be a major amount, such as greater than about 50 wt. %, greater than about 60 wt. %, greater than about 70 wt. %, greater than about 80 wt. %, greater than about 85 wt. %, or greater than about 90 wt. %.

## Antioxidants

The lubricating oil compositions herein also may optionally contain one or more antioxidants. Antioxidant compounds are known and include for example, phenates, phenate sulfides, sulfurized olefins, phosphosulfurized terpenes, sulfurized esters, aromatic amines, alkylated diphenylamines (e.g., nonyl diphenylamine, di-nonyl diphenylamine, octyl diphenylamine, di-octyl diphenylamine), phenyl-alpha-naphthylamines, alkylated phenyl-alpha-naphthylamines, hindered non-aromatic amines, phenols, hindered phenols, oil-soluble molybdenum compounds, macromolecular antioxidants, or mixtures thereof. Antioxidant compounds may be used alone or in combination.

The hindered phenol antioxidant may contain a secondary butyl and/or a tertiary butyl group as a sterically hindering group. The phenol group may be further substituted with a hydrocarbyl group and/or a bridging group linking to a second aromatic group. Examples of suitable hindered phenol antioxidants include 2,6-di-tert-butylphenol, 4-methyl-2,6-di-tert-butylphenol, 4-ethyl-2,6-di-tert-butylphenol, 4-propyl-2,6-di-tert-butylphenol or 4-butyl-2,6-di-tert-butylphenol, or 4-dodecyl-2,6-di-tert-butylphenol. In one embodiment the hindered phenol antioxidant may be an ester and may include, e.g., Irganox<sup>TM</sup> L-135 available from BASF or an addition product derived from 2,6-di-tert-butylphenol and an alkyl acrylate, wherein the alkyl group may contain about 1 to about 18, or about 2 to about 12, or about 2 to about 8, or about 2 to about 6, or about 4 carbon atoms. Another commercially available hindered phenol antioxidant may be an ester and may include Ethanox<sup>TM</sup> 4716 available from Albemarle Corporation.

Useful antioxidants may include diarylamines and high molecular weight phenols. In an embodiment, the lubricating oil composition may contain a mixture of a diarylamine and a high molecular weight phenol, such that each antioxidant may be present in an amount sufficient to provide up to about 5%, by weight, based upon the final weight of the lubricating oil composition. In an embodiment, the antioxidant may be a mixture of about 0.3 to about 1.5% diarylamine and about 0.4 to about 2.5% high molecular weight phenol, by weight, based upon the final weight of the lubricating oil composition.

Examples of suitable olefins that may be sulfurized to form a sulfurized olefin include propylene, butylene, isobutylene, polyisobutylene, pentene, hexene, heptene, octene, nonene, decene, undecene, dodecene, tridecene, tetradecene, pentadecene, hexadecene, heptadecene, octadecene, nonadecene, eicosene or mixtures thereof. In one embodiment, hexadecene, heptadecene, octadecene, nonadecene, eicosene or mixtures thereof and their dimers, trimers and tetramers are especially useful olefins. Alternatively, the olefin may be a Diels-Alder adduct of a diene such as 1,3-butadiene and an unsaturated ester, such as, butylacrylate.

Another class of sulfurized olefin includes sulfurized fatty acids and their esters. The fatty acids are often obtained from vegetable oil or animal oil and typically contain about 4 to about 22 carbon atoms. Examples of suitable fatty acids and their esters include triglycerides, oleic acid, linoleic acid, palmitoleic acid or mixtures thereof. Often, the fatty acids are obtained from lard oil, tall oil, peanut oil, soybean oil, cottonseed oil, sunflower seed oil or mixtures thereof. Fatty acids and/or ester may be mixed with olefins, such as, ct-olefins.

In another alternative embodiment the antioxidant composition also contains a molybdenum-containing antioxidant in addition to the phenolic and/or aminic antioxidants dis-

cussed above. When a combination of these three antioxidants is used, preferably the ratio of phenolic to aminic to molybdenum-containing is (0 to 2):(0 to 2):(0 to 1).

The one or more antioxidant(s) may be present in ranges about 0 wt. % to about 20 wt. %, or about 0.1 wt. % to about 10 wt. %, or about 1 wt. % to about 5 wt. %, of the lubricating oil composition.

## Antiwear Agents

The lubricating oil compositions herein also may optionally contain one or more antiwear agents. Examples of suitable antiwear agents include, but are not limited to, a metal thiophosphate; a metal dialkyldithiophosphate; a phosphoric acid ester or salt thereof; a phosphate ester(s); a phosphite; a phosphorus-containing carboxylic ester, ether, or amide; a sulfurized olefin; thiocarbamate-containing compounds including, thiocarbamate esters, alkylene-coupled thiocarbamates, and bis(S-alkyldithiocarbamyl)disulfides; and mixtures thereof. A suitable antiwear agent may be a molybdenum dithiocarbamate. The phosphorus containing antiwear agents are more fully described in European Patent 612 839. The metal in the dialkyl dithio phosphate salts may be an alkali metal, alkaline earth metal, aluminum, lead, tin, molybdenum, manganese, nickel, copper, titanium, or zinc. A useful antiwear agent may be zinc dialkyldithiophosphate.

Further examples of suitable antiwear agents include titanium compounds, tartrates, tartrimides, oil soluble amine salts of phosphorus compounds, sulfurized olefins, phosphites (such as dibutyl phosphite), phosphonates, thiocarbamate-containing compounds, such as thiocarbamate esters, thiocarbamate amides, thiocarbamic ethers, alkylene-coupled thiocarbamates, and bis(S-alkyldithiocarbamyl)disulfides. The tartrate or tartrimide may contain alkyl-ester groups, where the sum of carbon atoms on the alkyl groups may be at least 8. The antiwear agent may in one embodiment include a citrate.

The antiwear agent may be present in ranges including about 0 wt. % to about 15 wt. %, or about 0.01 wt. % to about 10 wt. %, or about 0.05 wt. % to about 5 wt. %, or about 0.1 wt. % to about 3 wt. % of the lubricating oil composition.

## Boron-Containing Compounds

The lubricating oil compositions herein may optionally contain one or more boron-containing compounds.

Examples of boron-containing compounds include borate esters, borated fatty amines, borated epoxides, borated detergents, and borated dispersants, such as borated succinimide dispersants, as disclosed in U.S. Pat. No. 5,883,057.

The boron-containing compound, if present, can be used in an amount sufficient to provide up to about 8 wt. %, about 0.01 wt. % to about 7 wt. %, about 0.05 wt. % to about 5 wt. %, or about 0.1 wt. % to about 3 wt. % of the lubricating oil composition.

In some embodiments, the boron-containing compound may be present in the lubricating oil composition as a borated succinimide dispersant. The lubricating oil composition may have from about 5 ppmw of boron to about 300 ppmw of boron, or from about 250 ppmw of boron or less, or from about 150 ppmw of boron or less, or from about 80 ppmw of boron or less, or from about 40 ppm of boron or less, or about 5 ppmw of boron or greater, or about 10 ppmw of boron or greater from the borated succinimide dispersant, based on the total weight of the lubricating oil composition. Detergents

The lubricating oil composition may optionally further comprise one or more neutral, low based, or overbased detergents, and mixtures thereof. Suitable detergent sub-

strates include phenates, sulfur containing phenates, sulfonates, calixarates, salixarates, salicylates, carboxylic acids, phosphorus acids, mono- and/or di-thiophosphoric acids, alkyl phenols, sulfur coupled alkyl phenol compounds, or methylene bridged phenols. Suitable detergents and their methods of preparation are described in greater detail in numerous patent publications, including U.S. Pat. No. 7,732,390 and references cited therein.

The detergent substrate may be salted with an alkali or alkaline earth metal such as, but not limited to, calcium, magnesium, potassium, sodium, lithium, barium, or mixtures thereof. In some embodiments, the detergent is free of barium. In some embodiments, a detergent may contain traces of other metals such as magnesium or calcium in amounts such as 50 ppm or less, 40 ppm or less, 30 ppm or less, 20 ppm or less, or 10 ppm or less. A suitable detergent may include alkali or alkaline earth metal salts of petroleum sulfonic acids and long chain mono- or di-alkylarylsulfonic acids with the aryl group being benzyl, tolyl, and xylyl. Examples of suitable detergents include, but are not limited to, calcium phenates, calcium sulfur containing phenates, calcium sulfonates, calcium calixarates, calcium salixarates, calcium salicylates, calcium carboxylic acids, calcium phosphorus acids, calcium mono- and/or di-thiophosphoric acids, calcium alkyl phenols, calcium sulfur coupled alkyl phenol compounds, calcium methylene bridged phenols, magnesium phenates, magnesium sulfur containing phenates, magnesium sulfonates, magnesium calixarates, magnesium salixarates, magnesium salicylates, magnesium carboxylic acids, magnesium phosphorus acids, magnesium mono- and/or di-thiophosphoric acids, magnesium alkyl phenols, magnesium sulfur coupled alkyl phenol compounds, magnesium methylene bridged phenols, sodium phenates, sodium sulfur containing phenates, sodium sulfonates, sodium calixarates, sodium salixarates, sodium salicylates, sodium carboxylic acids, sodium phosphorus acids, sodium mono- and/or di-thiophosphoric acids, sodium alkyl phenols, sodium sulfur coupled alkyl phenol compounds, or sodium methylene bridged phenols.

Overbased detergent additives are well known in the art and may be alkali or alkaline earth metal overbased detergent additives. Such detergent additives may be prepared by reacting a metal oxide or metal hydroxide with a substrate and carbon dioxide gas. The substrate is typically an acid, for example, an acid such as an aliphatic substituted sulfonic acid, an aliphatic substituted carboxylic acid, or an aliphatic substituted phenol.

The terminology "overbased" or "low-based/neutral" relates to metal salts, such as metal salts of sulfonates, carboxylates, and phenates, wherein the amount of metal present exceeds the stoichiometric amount. Such salts may have a conversion level in excess of 100% (i.e., they may comprise more than 100% of the theoretical amount of metal needed to convert the acid to its "normal," "neutral" salt). The expression "metal ratio," often abbreviated as MR, is used to designate the ratio of total chemical equivalents of metal in the overbased salt to chemical equivalents of the metal in a neutral salt according to known chemical reactivity and stoichiometry. In a normal or neutral salt, the metal ratio is one and in an overbased salt, MR, is greater than one. They are commonly referred to as overbased, hyperbased, or superbased salts and may be salts of organic sulfur acids, carboxylic acids, or phenols.

An overbased detergent of the lubricating oil composition may have a total base number (TBN) of about 200 mg KOH/gram or greater, or as further examples, about 250 mg

KOH/gram or greater, or about 350 mg KOH/gram or greater, or about 375 mg KOH/gram or greater, or about 400 mg KOH/gram or greater.

Examples of suitable overbased detergents include, but are not limited to, overbased calcium phenates, overbased calcium sulfur containing phenates, overbased calcium sulfonates, overbased calcium calixarates, overbased calcium salixarates, overbased calcium salicylates, overbased calcium carboxylic acids, overbased calcium phosphorus acids, overbased calcium mono- and/or di-thiophosphoric acids, overbased calcium alkyl phenols, overbased calcium sulfur coupled alkyl phenol compounds, overbased calcium methylene bridged phenols, overbased magnesium phenates, overbased magnesium sulfur containing phenates, overbased magnesium sulfonates, overbased magnesium calixarates, overbased magnesium salixarates, overbased magnesium salicylates, overbased magnesium carboxylic acids, overbased magnesium phosphorus acids, overbased magnesium mono- and/or di-thiophosphoric acids, overbased magnesium alkyl phenols, overbased magnesium sulfur coupled alkyl phenol compounds, or overbased magnesium methylene bridged phenols.

The overbased calcium phenate detergents have a total base number of at least about 150 mg KOH/g, at least about 225 mg KOH/g, at least about 225 mg KOH/g to about 400 mg KOH/g, at least about 225 mg KOH/g to about 350 mg KOH/g or about 230 mg KOH/g to about 350 mg KOH/g, all as measured by the method of ASTM D-2896. When such detergent compositions are formed in an inert diluent, e.g. a process oil, usually a mineral oil, the total base number reflects the basicity of the overall composition including diluent, and any other materials (e.g., promoter, etc.) that may be contained in the detergent composition.

The overbased detergent may have a metal to substrate ratio of from 1.1:1, or from 2:1, or from 4:1, or from 5:1, or from 7:1, or from 10:1.

A low-based/neutral detergent of the lubricating oil composition may have a total base number (TBN) of less than or equal to about 175 mg KOH/gram, or as further examples, about 150 mg KOH/gram or less, or about 350 mg KOH/gram or greater, or about 375 mg KOH/gram or greater, or about 400 mg KOH/gram or greater.

Examples of suitable low-based/neutral detergents include but are not limited to low-based/neutral calcium sulfonate detergent, low-based/neutral calcium salicylate detergent, or any combination thereof.

Suitable low-based/neutral calcium alkylbenzene sulfonate detergent compositions, most preferably low based calcium propylene-derived alkylaryl sulfonates are formed by preparing an alkali or alkaline earth metal salt of an alkylbenzene sulfonic acid and if desired, subjecting the salt in the presence of a small excess of an alkali or alkaline earth metal base such as an oxide, hydroxide, or alcoholate to the action of an acidic material such as carbon dioxide so that a small amount of overbasing occurs. This controlled overbasing can be conducted using the same materials in much the same way as the overbasing described above, of course the amount of metal base is such that the desired total base number of the sultant composition is achieved. Low-based/neutral calcium sulfurized alkylphenates are also suitable components in the compositions of this disclosure.

In some embodiments, a detergent is effective at reducing or preventing rust in an engine.

The detergent may be present at about 0 wt. % to about 10 wt. %, or about 0.1 wt. % to about 8 wt. %, or about 1 wt. % to about 4 wt. %, or greater than about 4 wt. % to about 8 wt. %.

In some embodiments, the lubricating oil composition includes a calcium-sulfonate detergent. The calcium-sulfonate detergent may be selected from overbased and low-based/neutral. In some embodiments, the lubricating oil composition includes from about 300 ppmw calcium to about 2500 ppmw calcium, or from about 400 ppmw calcium to about 2000 ppmw calcium, or from about 500 ppmw calcium to about 1800 ppmw calcium, or from about 500 ppmw calcium to about 1200 ppmw calcium, or from about 1200 ppmw calcium or less from the calcium-sulfonate detergent, based on the total weight of the lubricating oil composition.

#### Dispersants

The lubricating oil composition may optionally further comprise one or more dispersants or mixtures thereof. Dispersants are often known as ashless-type dispersants because, prior to mixing in a lubricating oil composition, they do not contain ash-forming metals and they do not normally contribute any ash when added to a lubricant. Ashless type dispersants are characterized by a polar group attached to a relatively high molecular weight hydrocarbon chain. Typical ashless dispersants include N-substituted long chain alkenyl succinimides. Examples of N-substituted long chain alkenyl succinimides include polyisobutylene succinimide with the number average molecular weight of the polyisobutylene substituent being in the range about 350 to about 50,000, or to about 5,000, or to about 3,000, as measured by GPC. Succinimide dispersants and their preparation are disclosed, for instance in U.S. Pat. Nos. 7,897,696 or 4,234,435. The polyolefin may be prepared from polymerizable monomers containing about 2 to about 16, or about 2 to about 8, or about 2 to about 6 carbon atoms. Succinimide dispersants are typically the imide formed from a polyamine, typically a poly(ethyleneamine)

Preferred amines are selected from polyamines and hydroxyamines. Examples of polyamines that may be used include, but are not limited to, diethylene triamine (DETA), triethylene tetramine (TETA), tetraethylene pentamine (TEPA), and higher homologues such as pentaethylene hexamine (PEHA), and the like.

A suitable heavy polyamine is a mixture of polyalkylene polyamines comprising small amounts of lower polyamine oligomers such as TEPA and PEHA (pentaethylene hexamine) but primarily oligomers with 6 or more nitrogen atoms, 2 or more primary amines per molecule, and more extensive branching than conventional polyamine mixtures. A heavy polyamine preferably includes polyamine oligomers containing 7 or more nitrogens per molecule and with 2 or more primary amines per molecule. The heavy polyamine comprises more than 28 wt. % (e.g. >32 wt. %) total nitrogen and an equivalent weight of primary amine groups of 120-160 grams per equivalent.

Suitable polyamines are commonly known as PAM and contain a mixture of ethylene amines where TEPA and pentaethylene hexamine (PEHA) are the major part of the polyamine, usually less than about 80%.

Typically, PAM has 8.7-8.9 milliequivalents of primary amine per gram (an equivalent weight of 115 to 112 grams per equivalent of primary amine) and a total nitrogen content of about 33-34 wt. %. Heavier cuts of PAM oligomers with practically no TEPA and only very small amounts of PEHA but containing primarily oligomers with more than 6 nitrogens and more extensive branching, may produce dispersants with improved dispersancy.

In an embodiment the present disclosure further comprises at least one polyisobutylene succinimide dispersant derived from polyisobutylene with a number average

molecular weight in the range about 350 to about 50,000, or to about 5000, or to about 3000, as determined by GPC. The polyisobutylene succinimide may be used alone or in combination with other dispersants.

In some embodiments, polyisobutylene, when included, may have greater than 50 mol %, greater than 60 mol %, greater than 70 mol %, greater than 80 mol %, or greater than 90 mol % content of terminal double bonds. Such PIB is also referred to as highly reactive PIB ("HR-PIB"). HR-PIB having a number average molecular weight ranging from about 800 to about 5000, as determined by GPC, is suitable for use in embodiments of the present disclosure. Conventional PIB typically has less than 50 mol %, less than 40 mol %, less than 30 mol %, less than 20 mol %, or less than 10 mol % content of terminal double bonds.

An HR-PIB having a number average molecular weight ranging from about 900 to about 3000 may be suitable, as determined by GPC. Such HR-PIB is commercially available, or can be synthesized by the polymerization of isobutene in the presence of a non-chlorinated catalyst such as boron trifluoride, as described in U.S. Pat. No. 4,152,499 to Boerzel, et al. and U.S. Pat. No. 5,739,355 to Gateau, et al. When used in the aforementioned thermal ene reaction, HR-PIB may lead to higher conversion rates in the reaction, as well as lower amounts of sediment formation, due to increased reactivity. A suitable method is described in U.S. Pat. No. 7,897,696.

In one embodiment the present disclosure further comprises at least one dispersant derived from polyisobutylene succinic anhydride ("PIBSA"). The PIBSA may have an average of between about 1.0 and about 2.0 succinic acid moieties per polymer.

The % actives of the alkenyl or alkyl succinic anhydride can be determined using a chromatographic technique. This method is described in column 5 and 6 in U.S. Pat. No. 5,334,321.

The percent conversion of the polyolefin is calculated from the % actives using the equation in column 5 and 6 in U.S. Pat. No. 5,334,321.

Unless stated otherwise, all percentages are in weight percent and all molecular weights are number average molecular weights determined by gel permeation chromatography (GPC) using commercially available polystyrene standards (with a number average molecular weight of 180 to about 18,000 as the calibration reference).

In one embodiment, the dispersant may be derived from a polyalphaolefin (PAO) succinic anhydride.

In one embodiment, the dispersant may be derived from olefin maleic anhydride copolymer. As an example, the dispersant may be described as a poly-PIBSA.

In an embodiment, the dispersant may be derived from an anhydride which is grafted to an ethylene-propylene copolymer.

A suitable class of nitrogen-containing dispersants may be derived from olefin copolymers (OCP), more specifically, ethylene-propylene dispersants which may be grafted with maleic anhydride. A more complete list of nitrogen-containing compounds that can be reacted with the functionalized OCP are described in U.S. Pat. Nos. 7,485,603; 7,786,057; 7,253,231; 6,107,257; and 5,075,383; and/or are commercially available.

The hydrocarbyl moiety of the hydrocarbyl-dicarboxylic acid or anhydride of Component A) may alternatively be derived from ethylene-alpha olefin copolymers. These copolymers contain a plurality of ethylene units and a plurality of one or more C<sub>3</sub>-C<sub>10</sub> alpha-olefin units. The C<sub>3</sub>-C<sub>10</sub> alpha-olefin units may include propylene units.

One class of suitable dispersants may be Mannich bases. Mannich bases are materials that are formed by the condensation of a higher molecular weight, alkyl substituted phenol, a polyalkylene polyamine, and an aldehyde such as formaldehyde. Mannich bases are described in more detail in U.S. Pat. No. 3,634,515.

A suitable class of dispersants may be high molecular weight esters or half ester amides.

A suitable dispersant may also be post-treated by conventional methods by a reaction with any of a variety of agents. Among these are boron, urea, thiourea, dimercaptothiadiazoles, carbon disulfide, aldehydes, ketones, carboxylic acids, hydrocarbon-substituted succinic anhydrides, maleic anhydride, nitriles, epoxides, carbonates, cyclic carbonates, hindered phenolic esters, and phosphorus compounds. U.S. Pat. Nos. 7,645,726; 7,214,649; and 8,048,831 are incorporated herein by reference in their entireties.

In addition to the carbonate and boric acids post-treatments both the compounds may be post-treated, or further post-treatment, with a variety of post-treatments designed to improve or impart different properties. Such post-treatments include those summarized in columns 27-29 of U.S. Pat. No. 5,241,003, hereby incorporated by reference. Such treatments include, treatment with:

Inorganic phosphorous acids or anhydrides (e.g., U.S. Pat. Nos. 3,403,102 and 4,648,980); Organic phosphorous compounds (e.g., U.S. Pat. No. 3,502,677); Phosphorous pentasulfides;

Boron compounds as already noted above (e.g., U.S. Pat. Nos. 3,178,663 and 4,652,387);

Carboxylic acid, polycarboxylic acids, anhydrides and/or acid halides (e.g., U.S. Pat. Nos. 3,708,522 and 4,948,386);

Epoxides polyepoxides or thioepoxides (e.g., U.S. Pat. Nos. 3,859,318 and 5,026,495);

Aldehyde or ketone (e.g., U.S. Pat. No. 3,458,530);

Carbon disulfide (e.g., U.S. Pat. No. 3,256,185);

Glycidol (e.g., U.S. Pat. No. 4,617,137);

Urea, thourea or guanidine (e.g., U.S. Pat. Nos. 3,312,619; 3,865,813; and British Patent GB 1,065,595);

Organic sulfonic acid (e.g., U.S. Pat. No. 3,189,544 and British Patent GB 2,140,811);

Alkenyl cyanide (e.g., U.S. Pat. Nos. 3,278,550 and 3,366,569);

Diketene (e.g., U.S. Pat. No. 3,546,243);

A diisocyanate (e.g., U.S. Pat. No. 3,573,205);

Alkane sultone (e.g., U.S. Pat. No. 3,749,695);

1,3-Dicarbonyl Compound (e.g., U.S. Pat. No. 4,579,675);

Sulfate of alkoxylated alcohol or phenol (e.g., U.S. Pat. No. 3,954,639);

Cyclic lactone (e.g., U.S. Pat. Nos. 4,617,138; 4,645,515; 4,668,246; 4,963,275; and 4,971,711);

Cyclic carbonate or thiocarbonate linear monocarbonate or polycarbonate, or chloroformate (e.g., U.S. Pat. Nos. 4,612,132; 4,647,390; 4,648,886; 4,670,170);

Nitrogen-containing carboxylic acid (e.g., U.S. Pat. 4,971,598 and British Patent GB 2,140,811);

Hydroxy-protected chlorodicarbonyloxy compound (e.g., U.S. Pat. No. 4,614,522);

Lactam, thiolactam, thiolactone or dithiolactone (e.g., U.S. Pat. Nos. 4,614,603 and 4,666,460);

Cyclic carbonate or thiocarbonate, linear monocarbonate or polycarbonate, or chloroformate (e.g., U.S. Pat. Nos. 4,612,132; 4,647,390; 4,646,860; and 4,670,170);

Nitrogen-containing carboxylic acid (e.g., U.S. Pat. No. 4,971,598 and British Patent GB 2,440,811);

Hydroxy-protected chlorodicarbonyloxy compound (e.g., U.S. Pat. No. 4,614,522);

Lactam, thiolactam, thiolactone or dithiolactone (e.g., U.S. Pat. Nos. 4,614,603, and 4,666,460);

5 Cyclic carbamate, cyclic thiocarbamate or cyclic dithiocarbamate (e.g., U.S. Pat. Nos. 4,663,062 and 4,666,459);

Hydroxyaliphatic carboxylic acid (e.g., U.S. Pat. Nos. 4,482,464; 4,521,318; 4,713,189);

Oxidizing agent (e.g., U.S. Pat. No. 4,379,064);

10 Combination of phosphorus pentasulfide and a polyalkylene polyamine (e.g., U.S. Pat. No. 3,185,647);

Combination of carboxylic acid or an aldehyde or ketone and sulfur or sulfur chloride (e.g., U.S. Pat. Nos. 3,390,086; 3,470,098);

15 Combination of a hydrazine and carbon disulfide (e.g. U.S. Pat. No. 3,519,564);

Combination of an aldehyde and a phenol (e.g., U.S. Pat. Nos. 3,649,229; 5,030,249; 5,039,307); Combination of an aldehyde and an O-diester of dithiophosphoric acid (e.g., U.S. Pat. No. 3,865,740);

20 Combination of a hydroxyaliphatic carboxylic acid and a boric acid (e.g., U.S. Pat. No. 4,554,086);

Combination of a hydroxyaliphatic carboxylic acid, then formaldehyde and a phenol (e.g., U.S. Pat. No. 4,636,322);

25 Combination of a hydroxyaliphatic carboxylic acid and then an aliphatic dicarboxylic acid (e.g., U.S. Pat. No. 4,663,064);

Combination of formaldehyde and a phenol and then glycolic acid (e.g., U.S. Pat. No. 4,699,724);

30 Combination of a hydroxyaliphatic carboxylic acid or oxalic acid and then a diisocyanate (e.g. U.S. Pat. No. 4,713,191);

Combination of inorganic acid or anhydride of phosphorus or a partial or total sulfur analog thereof and a boron compound (e.g., U.S. Pat. No. 4,857,214);

35 Combination of an organic diacid then an unsaturated fatty acid and then a nitrosoaromatic amine optionally followed by a boron compound and then a glycolating agent (e.g., U.S. Pat. No. 4,973,412);

40 Combination of an aldehyde and a triazole (e.g., U.S. Pat. No. 4,963,278);

Combination of an aldehyde and a triazole then a boron compound (e.g., U.S. Pat. No. 4,981,492);

45 Combination of cyclic lactone and a boron compound (e.g., U.S. Pat. No. 4,963,275 and 4,971,711). The above-mentioned patents are herein incorporated in their entireties.

The TBN of a suitable dispersant may be from about 10 to about 65 mg KOH/g dispersant, on an oil-free basis, which is comparable to about 5 to about 30 TBN if measured on a dispersant sample containing about 50% diluent oil. TBN is measured by the method of ASTM D2896.

The dispersant, if present, can be used in an amount sufficient to provide up to about 20 wt. %, based upon the final weight of the lubricating oil composition. Another amount of the dispersant that can be used may be about 0.1 wt. % to about 15 wt. %, or about 0.1 wt. % to about 10 wt. %, or about 3 wt. % to about 10 wt. %, or about 1 wt. % to about 6 wt. %, or about 7 wt. % to about 12 wt. %, based upon the final weight of the lubricating oil composition. In some embodiments, the lubricating oil composition utilizes a mixed dispersant system. A single type or a mixture of two or more types of dispersants in any desired ratio may be used.

#### Friction Modifiers

60 The lubricating oil compositions herein also may optionally contain one or more friction modifiers. Suitable friction modifiers may comprise metal containing and metal-free

friction modifiers and may include, but are not limited to, imidazolines, amides, amines, succinimides, alkoxylated amines, alkoxylated ether amines, amine oxides, amidoamines, nitriles, betaines, quaternary amines, imines, amine salts, amino guanadine, alkanolamides, phosphonates, metal-containing compounds, glycerol esters, sulfurized fatty compounds and olefins, sunflower oil other naturally occurring plant or animal oils, dicarboxylic acid esters, esters or partial esters of a polyol and one or more aliphatic or aromatic carboxylic acids, and the like.

Suitable friction modifiers may contain hydrocarbyl groups that are selected from straight chain, branched chain, or aromatic hydrocarbyl groups or mixtures thereof, and may be saturated or unsaturated. The hydrocarbyl groups may be composed of carbon and hydrogen or hetero atoms such as sulfur or oxygen. The hydrocarbyl groups may range from about 12 to about 25 carbon atoms. In some embodiments the friction modifier may be a long chain fatty acid ester. In another embodiment the long chain fatty acid ester may be a mono-ester, or a di-ester, or a (tri)glyceride. The friction modifier may be a long chain fatty amide, a long chain fatty ester, a long chain fatty epoxide derivatives, or a long chain imidazoline.

Other suitable friction modifiers may include organic, ashless (metal-free), nitrogen-free organic friction modifiers. Such friction modifiers may include esters formed by reacting carboxylic acids and anhydrides with alkanols and generally include a polar terminal group (e.g. carboxyl or hydroxyl) covalently bonded to an oleophilic hydrocarbon chain. An example of an organic ashless nitrogen-free friction modifier is known generally as glycerol monooleate (GMO) which may contain mono-, di-, and tri-esters of oleic acid. Other suitable friction modifiers are described in U.S. Pat. No. 6,723,685, herein incorporated by reference in its entirety.

Aminic friction modifiers may include amines or polyamines. Such compounds can have hydrocarbyl groups that are linear, either saturated or unsaturated, or a mixture thereof and may contain from about 12 to about 25 carbon atoms. Further examples of suitable friction modifiers include alkoxylated amines and alkoxylated ether amines. Such compounds may have hydrocarbyl groups that are linear, either saturated, unsaturated, or a mixture thereof. They may contain from about 12 to about 25 carbon atoms. Examples include ethoxylated amines and ethoxylated ether amines.

The amines and amides may be used as such or in the form of an adduct or reaction product with a boron compound such as a boric oxide, boron halide, metaborate, boric acid or a mono-, di- or tri-alkyl borate. Other suitable friction modifiers are described in U.S. Pat. No. 6,300,291, herein incorporated by reference in its entirety.

A friction modifier may optionally be present in ranges such as about 0 wt. % to about 10 wt. %, or about 0.01 wt. % to about 8 wt. %, or about 0.1 wt. % to about 4 wt. %.

Molybdenum-Containing Component

The lubricating oil compositions herein also may optionally contain one or more molybdenum-containing compounds. An oil-soluble molybdenum compound may have the functional performance of an antiwear agent, an antioxidant, a friction modifier, or mixtures thereof. An oil-soluble molybdenum compound may include molybdenum dithiocarbamates, molybdenum dialkyldithiophosphates, molybdenum dithiophosphinates, amine salts of molybdenum compounds, molybdenum xanthates, molybdenum thioxanthates, molybdenum sulfides, molybdenum carboxylates, molybdenum alkoxides, a trinuclear organo-molybde-

num compound, and/or mixtures thereof. The molybdenum sulfides include molybdenum disulfide. The molybdenum disulfide may be in the form of a stable dispersion. In one embodiment the oil-soluble molybdenum compound may be selected from the group consisting of molybdenum dithiocarbamates, molybdenum dialkyldithiophosphates, amine salts of molybdenum compounds, and mixtures thereof. In one embodiment the oil-soluble molybdenum compound may be a molybdenum dithiocarbamate.

10 Suitable examples of molybdenum compounds which may be used include commercial materials sold under the trade names such as Molyvan 822<sup>TM</sup>, Molyvan<sup>TM</sup> A, Molyvan 2000<sup>TM</sup> and Molyvan 855<sup>TM</sup> from R. T. Vanderbilt Co., Ltd., and Sakura-Lube<sup>TM</sup> S-165, S-200, S-300, 5-310G, 15 S-525, S-600, S-700, and S-710 available from Adeka Corporation, and mixtures thereof. Suitable molybdenum components are described in U.S. Pat. No. 5,650,381; U.S. RE 37,363 E1; U.S. RE 38,929 E1; and U.S. RE 40,595 E1, incorporated herein by reference in their entireties.

20 Additionally, the molybdenum compound may be an acidic molybdenum compound. Included are molybdic acid, ammonium molybdate, sodium molybdate, potassium molybdate, and other alkaline metal molybdates and other molybdenum salts, e.g., hydrogen sodium molybdate, 25 MoOCl<sub>4</sub>, MoO<sub>2</sub>Br<sub>2</sub>, Mo<sub>2</sub>O<sub>3</sub>Cl<sub>6</sub>, molybdenum trioxide or similar acidic molybdenum compounds. Alternatively, the compositions can be provided with molybdenum by molybdenum/sulfur complexes of basic nitrogen compounds as described, for example, in U.S. Pat. Nos. 4,263,152; 4,285, 30 822; 4,283,295; 4,272,387; 4,265,773; 4,261,843; 4,259,195 and 4,259,194; and WO 94/06897, incorporated herein by reference in their entireties.

Another class of suitable organo-molybdenum compounds are trinuclear molybdenum compounds, such as 35 those of the formula Mo<sub>3</sub>S<sub>k</sub>L<sub>n</sub>Q<sub>z</sub> and mixtures thereof, wherein S represents sulfur, L represents independently selected ligands having organo groups with a sufficient number of carbon atoms to render the compound soluble or dispersible in the oil, n is from 1 to 4, k varies from 4 through 7, Q is selected from the group of neutral electron 40 donating compounds such as water, amines, alcohols, phosphines, and ethers, and z ranges from 0 to 5 and includes non-stoichiometric values. At least 21 total carbon atoms may be present among all the ligands' organo groups, such as at least 25, at least 30, or at least 35 carbon atoms. Additional suitable molybdenum compounds are described in U.S. Pat. No. 6,723,685, herein incorporated by reference in its entirety.

The oil-soluble molybdenum compound may be present 50 in an amount sufficient to provide about 0.5 ppm to about 2000 ppm, about 1 ppm to about 700 ppm, about 1 ppm to about 550 ppm, about 5 ppm to about 300 ppm, or about 20 ppm to about 250 ppm of molybdenum.

#### Transition Metal-Containing Compounds

55 In another embodiment, the oil-soluble compound may be a transition metal containing compound or a metalloid. The transition metals may include, but are not limited to, titanium, vanadium, copper, zinc, zirconium, molybdenum, tantalum, tungsten, and the like. Suitable metalloids include, but are not limited to, boron, silicon, antimony, tellurium, and the like.

In an embodiment, an oil-soluble transition metal-containing compound may function as antiwear agents, friction modifiers, antioxidants, deposit control additives, or more than one of these functions. In an embodiment the oil-soluble transition metal-containing compound may be an oil-soluble titanium compound, such as a titanium (IV)

alkoxide. Among the titanium containing compounds that may be used in, or which may be used for preparation of the oils-soluble materials of, the disclosed technology are various Ti (IV) compounds such as titanium (IV) oxide; titanium (IV) sulfide; titanium (IV) nitrate; titanium (IV) alkoxides such as titanium methoxide, titanium ethoxide, titanium propoxide, titanium isopropoxide, titanium butoxide, titanium 2-ethylhexoxide; and other titanium compounds or complexes including but not limited to titanium phenates; titanium carboxylates such as titanium (IV) 2-ethyl-1-3-hexanedioate or titanium citrate or titanium oleate; and titanium (IV) (triethanolaminato)isopropoxide. Other forms of titanium encompassed within the disclosed technology include titanium phosphates such as titanium dithiophosphates (e.g., dialkyldithiophosphates) and titanium sulfonates (e.g., alkylbenzenesulfonates), or, generally, the reaction product of titanium compounds with various acid materials to form salts, such as oil-soluble salts. Titanium compounds can thus be derived from, among others, organic acids, alcohols, and glycols. Ti compounds may also exist in dimeric or oligomeric form, containing Ti—O—Ti structures. Such titanium materials are commercially available or can be readily prepared by appropriate synthesis techniques which will be apparent to the person skilled in the art. They may exist at room temperature as a solid or a liquid, depending on the particular compound. They may also be provided in a solution form in an appropriate inert solvent.

In one embodiment, the titanium can be supplied as a Ti-modified dispersant, such as a succinimide dispersant. Such materials may be prepared by forming a titanium mixed anhydride between a titanium alkoxide and a hydrocarbyl-substituted succinic anhydride, such as an alkenyl- (or alkyl) succinic anhydride. The resulting titanate-succinate intermediate may be used directly or it may be reacted with any of a number of materials, such as (a) a polyamine-based succinimide/amide dispersant having free, condensable —NH functionality; (b) the components of a polyamine-based succinimide/amide dispersant, i.e., an alkenyl- (or alkyl-) succinic anhydride and a polyamine, (c) a hydroxy-containing polyester dispersant prepared by the reaction of a substituted succinic anhydride with a polyol, aminoalcohol, polyamine, or mixtures thereof. Alternatively, the titanate-succinate intermediate may be reacted with other agents such as alcohols, aminoalcohols, ether alcohols, polyether alcohols or polyols, or fatty acids, and the product thereof either used directly to impart Ti to a lubricant, or else further reacted with the succinic dispersants as described above. As an example, 1 part (by mole) of tetraisopropyl titanate may be reacted with about 2 parts (by mole) of a polyisobutene-substituted succinic anhydride at 140-150° C. for 5 to 6 hours to provide a titanium modified dispersant or intermediate. The resulting material (30 g) may be further reacted with a succinimide dispersant from polyisobutene-substituted succinic anhydride and a polyethylenepolyamine mixture (127 grams +diluent oil) at 150° C. for 1.5 hours, to produce a titanium-modified succinimide dispersant.

Another titanium containing compound may be a reaction product of titanium alkoxide and C<sub>6</sub> to C<sub>25</sub> carboxylic acid. The reaction product may be represented by the following formula:



wherein n is an integer selected from 2, 3 and 4, and R is a hydrocarbyl group containing from about 5 to about 24 carbon atoms, or by the formula:



wherein m+n=4 and n ranges from 1 to 3, R<sub>4</sub> is an alkyl moiety with carbon atoms ranging from 1-8, R<sub>1</sub> is selected from a hydrocarbyl group containing from about 6 to 25 carbon atoms, and R<sub>2</sub> and R<sub>3</sub> are the same or different and are selected from a hydrocarbyl group containing from about 1 to 6 carbon atoms, or the titanium compound may be represented by the formula:



wherein x ranges from 0 to 3, R<sub>1</sub> is selected from a hydrocarbyl group containing from about 6 to 25 carbon atoms, R<sub>2</sub>, and R<sub>3</sub> are the same or different and are selected from a hydrocarbyl group containing from about 1 to 6 carbon atoms, and R<sub>4</sub> is selected from a group consisting of either H, or C<sub>6</sub> to C<sub>25</sub> carboxylic acid moiety.

Suitable carboxylic acids may include, but are not limited to caproic acid, caprylic acid, lauric acid, myristic acid, palmitic acid, stearic acid, arachidic acid, oleic acid, erucic acid, linoleic acid, linolenic acid, cyclohexanecarboxylic acid, phenylacetic acid, benzoic acid, neodecanoic acid, and the like.

In an embodiment the oil soluble titanium compound may be present in the lubricating oil composition in an amount to provide from 0 to 3000 ppm titanium by weight or 25 to about 1500 ppm titanium by weight or about 35 ppm to 500 ppm titanium by weight or about 50 ppm to about 300 ppm. Viscosity Index Improvers

The lubricating oil compositions herein also may optionally contain one or more viscosity index improvers. Suitable viscosity index improvers may include polyolefins, olefin copolymers, ethylene/propylene copolymers, polyisobutenes, hydrogenated styrene-isoprene polymers, styrene/maleic ester copolymers, hydrogenated styrene/butadiene copolymers, hydrogenated isoprene polymers, alpha-olefin maleic anhydride copolymers, polymethacrylates, polyacrylates, polyalkyl styrenes, hydrogenated alkenyl aryl conjugated diene copolymers, or mixtures thereof. Viscosity index improvers may include star polymers and suitable examples are described in US Publication No. 20120101017A1.

The lubricating oil compositions herein also may optionally contain one or more dispersant viscosity index improvers in addition to a viscosity index improver or in lieu of a viscosity index improver. Suitable viscosity index improvers may include functionalized polyolefins, for example, ethylene-propylene copolymers that have been functionalized with the reaction product of an acylating agent (such as maleic anhydride) and an amine; polymethacrylates functionalized with an amine, or esterified maleic anhydride-styrene copolymers reacted with an amine.

The total amount of viscosity index improver and/or dispersant viscosity index improver may be about 0 wt. % to about 20 wt. %, about 0.1 wt. % to about 15 wt. %, about 0.1 wt. % to about 12 wt. %, or about 0.5 wt. % to about 10 wt. %, of the lubricating oil composition.

#### Other Optional Additives

Other additives may be selected to perform one or more functions required of a lubricating fluid. Further, one or more of the mentioned additives may be multi-functional and provide functions in addition to or other than the function prescribed herein.

A lubricating oil composition according to the present disclosure may optionally comprise other performance additives. The other performance additives may be in addition to specified additives of the present disclosure and/or may comprise one or more of metal deactivators, viscosity index improvers, detergents, ashless TBN boosters, friction modifiers, antiwear agents, corrosion inhibitors, rust inhibitors, dispersants, dispersant viscosity index improvers, extreme pressure agents, antioxidants, foam inhibitors, demulsifiers, emulsifiers, pour point depressants, seal swelling agents and mixtures thereof. Typically, fully-formulated lubricating oil will contain one or more of these performance additives.

Suitable metal deactivators may include derivatives of benzotriazoles (typically tolyltriazole), dimercaptothiadiazole derivatives, 1,2,4-triazoles, benzimidazoles, 2-alkyldithiobenzimidazoles, or 2-alkyldithiobenzothiazoles; foam inhibitors including copolymers of ethyl acrylate and 2-ethylhexylacrylate and optionally vinyl acetate; demulsifiers including trialkyl phosphates, polyethylene glycols, poly-ethylene oxides, polypropylene oxides and (ethylene oxide-propylene oxide) polymers; pour point depressants including esters of maleic anhydride-styrene, polymethacrylates, polyacrylates or polyacrylamides.

Suitable foam inhibitors include silicon-based compounds, such as siloxane.

Suitable pour point depressants may include a polymethylmethacrylates or mixtures thereof. Pour point depressants may be present in an amount sufficient to provide from about 0 wt. % to about 1 wt. %, about 0.01 wt. % to about 0.5 wt. %, or about 0.02 wt. % to about 0.04 wt. % based upon the final weight of the lubricating oil composition.

Suitable rust inhibitors may be a single compound or a mixture of compounds having the property of inhibiting corrosion of ferrous metal surfaces. Non-limiting examples of rust inhibitors useful herein include oil-soluble high molecular weight organic acids, such as 2-ethylhexanoic acid, lauric acid, myristic acid, palmitic acid, oleic acid, linoleic acid, linolenic acid, behenic acid, and cerotic acid, as well as oil-soluble polycarboxylic acids including dimer and trimer acids, such as those produced from tall oil fatty acids, oleic acid, and linoleic acid. Other suitable corrosion inhibitors include long-chain alpha, omega-dicarboxylic acids in the molecular weight range of about 600 to about 3000 and alkenylsuccinic acids in which the alkenyl group contains about 10 or more carbon atoms such as, tetrapropenylsuccinic acid, tetradecenylsuccinic acid, and hexade-

cenylsuccinic acid. Another useful type of acidic corrosion inhibitors are the half esters of alkenyl succinic acids having about 8 to about 24 carbon atoms in the alkenyl group with alcohols such as the polyglycols. The corresponding half amides of such alkenyl succinic acids are also useful. A useful rust inhibitor is a high molecular weight organic acid. In some embodiments, an engine oil is devoid of a rust inhibitor.

The rust inhibitor, if present, can be used in an amount sufficient to provide about 0 wt. % to about 5 wt. %, about 0.01 wt. % to about 3 wt. %, about 0.1 wt. % to about 2 wt. %, based upon the final weight of the lubricating oil composition.

In general terms, a suitable crankcase lubricant may include additive components in the ranges listed in the following table.

TABLE 2

| Component                                              | Wt. %<br>(Broad) | Wt. %<br>(Typical) |
|--------------------------------------------------------|------------------|--------------------|
| Dispersant(s)                                          | 0.1-15.0         | 1.0-8.0            |
| Metal Detergent(s)                                     | 0.1-3.0          | 0.2-2.0            |
| Antioxidant(s)                                         | 0.1-4.0          | 0.01-2.0           |
| Detergent(s)                                           | 0.1-3.0          | 0.2-2.0            |
| Ashless TBN booster(s)                                 | 0.0-1.0          | 0.01-0.5           |
| Corrosion inhibitor(s)                                 | 0.0-2.0          | 0.0-0.5            |
| Metal dihydrocarbyl dithiophosphate(s)                 | 0.1-3.0          | 0.1-2.0            |
| Ash-free phosphorus compound(s)                        | 0.0-2.0          | 0.0-1.0            |
| Antifoaming agent(s)                                   | 0.0-1.0          | 0.001-0.15         |
| Antiwear agent(s)                                      | 0.0-1.0          | 0.0-0.8            |
| Pour point depressant(s)                               | 0.0-2.0          | 0.001-0.5          |
| Viscosity index improver(s) (on a liquid/dilute basis) | 0.0-20.0         | 0.1-15.0           |
| Dispersant viscosity index improver(s)                 | 0.0-10.0         | 0.0-5.0            |
| Friction modifier(s)                                   | 0.001-2.0        | 0.05-1.0           |
| Base oil(s)                                            | Balance          | Balance            |
| Total                                                  | 100              | 100                |

The percentages of each component above represent the weight percent of each component, based upon the weight of the final lubricating oil composition. The remainder of the lubricating oil composition consists of one or more base oils.

Additives used in formulating the compositions described herein may be blended into the base oil individually or in various sub-combinations. However, it may be suitable to blend all of the components concurrently using an additive concentrate (i.e., additives plus a diluent, such as a hydrocarbon solvent).

#### EXAMPLES

The following examples are illustrative, but not limiting, of the methods and compositions of the present disclosure. Other suitable modifications and adaptations of the variety of conditions and parameters normally encountered in the field, and which are obvious to those skilled in the art, are within the spirit and scope of the disclosure. All patents and publications cited herein are fully incorporated by reference herein in their entirety.

To demonstrate how the zinc dialkyl dithiophosphates may affect the properties of the lubricating oil composition in a hybrid engine, the lubricating oil compositions were tested for phosphorus retention and wear. Each of the foregoing examples included a succinimide dispersant(s), borated succinimide dispersant(s), organic friction modifier(s), molybdenum-containing compound(s) calcium sulfonate detergent(s), antioxidant(s), antifoam agent(s),

pour point depressant(s), and viscosity index improver(s), present in an amount according to Table 2.

To determine the amount of phosphorus volatilized during engine aging the amount of calcium and phosphorus in the unaged and aged oils was determined by inductively coupling plasma atomic emission spectroscopy (ICP). The phosphorus retention was calculated by determining the ratio of phosphorus in the aged oil versus phosphorus in the unaged oil, corrected for the amount of volatile base oil components released by the oil. The volatility correction is determined by the ratio of calcium in the aged oil to calcium in the unaged oil. An increase in calcium concentration indicates a loss in volatile components in the oil. The tracking of calcium concentration as an indication of loss of volatile base oil components is used in the Sequence IIIG protocol to determine phosphorus retention. This protocol may be found in more detail in *Engine Oil Performance and Engine Service Classification*, SAE J183, March 2006. The results for the phosphorus retention may be found in Table 3.

TABLE 3

| Example                                                                           | IE1   | IE2   | IE3   | IE4   |
|-----------------------------------------------------------------------------------|-------|-------|-------|-------|
| Molar Ratio of Primary to Secondary Alcohol of the ZDDP component                 | 0:100 | 60:40 | 100:0 | 100:0 |
| Average Number of Total Carbon Atoms per Mole of Phosphorus of the ZDDP component | 12    | 8.8   | 9.3   | 16    |
| Molar Ratio of Zn to P in ZDDP component                                          | 1.098 | 1.098 | 1.125 | 1.270 |
| Zn ppm from ZDDP component to finished fluid                                      | 892   | 821   | 821   | 821   |
| P ppm from ZDDP component to finished fluid                                       | 752   | 710   | 710   | 710   |
| Phosphorus retention after aging @ 70° C.                                         | 98%   | 100%  | 99%   | 103%  |
| Phosphorus retention after aging @ 150° C.                                        | 89%   | 77%   | 79%   | 97%   |

As seen from Table 3, each of Examples 1-4 included different ZDDP compounds which all provided improved phosphorus retention at operating temperatures of about 70° C., relative to the typical operating temperatures of typical internal combustion engines. Furthermore, the results of this test indicate that phosphorus from the ZDDP components volatilizes at a temperature of about 150° C. and greater, reflective of the operating temperatures of typical internal combustion engines. In contrast, little to no phosphorus volatilization of the ZDDP components was observed after aging to 70° C., reflective of the operating temperatures of a hybrid internal combustion engine. IE-4 demonstrated relatively good results at both 70° C. and 150° C., indicating that the ZDDP component did not reach degradation temperatures.

The lubricating oils which were aged at 70° C. and 150° C. were also tested using PCS Instruments' High Frequency Reciprocating Rig (HFRR) test to determine the effects of various ZDDP components on wear at various temperatures. In the HFRR tests, an ANSI 52100 steel ball was oscillated across an ANSI 52100 steel disk. The ball was oscillated at a speed of 20Hz over a two-millimeter path, with an applied load of 700g between the ball and the test surface. The tests were run for 60 minutes at a temperature of 120° C. The test conditions employed here have been used previously to

examine the wear prevention properties of engine oils with known wear performance in vehicle field tests, in the following articles: M. D. Johnson, S. Korcek, R. K. Jensen, A. K. Gangopadhyay and E. A. Sotis, *Laboratory Assessment of the Oxidation and Wear Performance Capabilities of Low Phosphorus Engine Oils*, SAE Technical Series Paper 2001-01-3541 (2001) and H. Gao, K. K. Bjornen, A. K. Gangopadhyay and R. K. Jensen, *Oxidation and Antiwear Retention Capability of Low-Phosphorus Engine Oils*, SAE Technical Series Paper 2005-01-3822 (2005). After testing, a surface trace of the wear scar on the test surface was measured using the MicroAnalyzer 2000 from Precision Devices Incorporated (PDI) and the area of the wear scar was recorded.

TABLE 4

| Example                                                                           | CE1   | CE2   | CE3   | IE5   |
|-----------------------------------------------------------------------------------|-------|-------|-------|-------|
| Ratio of Primary to Secondary Alcohol of the ZDDP component                       | 0:100 | 60:40 | 100:0 | 100:0 |
| Average Number of Total Carbon Atoms per Mole of Phosphorus of the ZDDP component | 12    | 8.8   | 9.3   | 16    |
| Ratio of Zn to P in ZDDP component                                                | 1.098 | 1.098 | 1.125 | 1.270 |
| Zn ppm from ZDDP component to finished fluid                                      | 892   | 821   | 821   | 821   |
| P ppm from ZDDP component to finished fluid                                       | 752   | 710   | 710   | 710   |
| HFRR wear after aging @ 70° C.                                                    | 173   | 228   | 132   | 66    |
| HFRR wear after aging @ 150° C.                                                   | 341   | 191   | 91    | 382   |

As seen from Table 4, the best results observed at operating conditions of about 70° C. were when the ZDDP component was derived from 100 mole percent of one or more primary alkyl alcohols or when it was derived from a ZDDP component having a molar ratio of Zn to P from the ZDDP component of 1.270 or greater. The best results were unexpected and were observed in Inventive Example 5 which employed a ZDDP component derived from 100 mole percent of one or more primary and a molar ratio of Zn to P from the ZDDP component of 1.270.

As observed in Table 4, ZDDP components derived from primary alcohols degrade at much higher temperatures than the operating conditions of hybrid internal combustion engines and typical internal combustion engines. ZDDP components have anti-wear properties which impart their protective properties when the ZDDP component is degraded and forms a film on metal surfaces. Based on Table 4, it was surprising that the lubricating oil composition Example IE-5 provided the best results in terms of wear protection, as Table 3 indicated that the ZDDP component derived from 100 mol % primary alcohols degrades at temperatures even higher than the operating temperature of a typical internal combustion engine.

Other embodiments of the present disclosure will be apparent to those skilled in the art from consideration of the specification and practice of the embodiments disclosed herein. As used throughout the specification and claims, "a" and/or "an" may refer to one or more than one. Unless otherwise indicated, all numbers expressing quantities of ingredients, properties such as molecular weight, percent, ratio, reaction conditions, and so forth used in the specifi-

31

cation and claims are to be understood as being modified in all instances by the term "about," whether or not the term "about" is present. Accordingly, unless indicated to the contrary, the numerical parameters set forth in the specification and claims are approximations that may vary depending upon the desired properties sought to be obtained by the present disclosure. At the very least, and not as an attempt to limit the application of the doctrine of equivalents to the scope of the claims, each numerical parameter should at least be construed in light of the number of reported significant digits and by applying ordinary rounding techniques. Notwithstanding that the numerical ranges and parameters setting forth the broad scope of the disclosure are approximations, the numerical values set forth in the specific examples are reported as precisely as possible. Any numerical value, however, inherently contains certain errors necessarily resulting from the standard deviation found in their respective testing measurements. It is intended that the specification and examples be considered as exemplary only, with a true scope and spirit of the disclosure being indicated by the following claims.

The foregoing embodiments are susceptible to considerable variation in practice. Accordingly, the embodiments are not intended to be limited to the specific exemplifications set forth hereinabove. Rather, the foregoing embodiments are within the spirit and scope of the appended claims, including the equivalents thereof available as a matter of law.

The patentees do not intend to dedicate any disclosed embodiments to the public, and to the extent any disclosed modifications or alterations may not literally fall within the scope of the claims, they are considered to be part hereof under the doctrine of equivalents.

It is to be understood that each component, compound, substituent or parameter disclosed herein is to be interpreted as being disclosed for use alone or in combination with one or more of each and every other component, compound, substituent or parameter disclosed herein.

It is also to be understood that each amount/value or range of amounts/values for each component, compound, substituent or parameter disclosed herein is to be interpreted as also being disclosed in combination with each amount/value or range of amounts/values disclosed for any other component(s), compounds(s), substituent(s) or parameter(s) disclosed herein and that any combination of amounts/values or ranges of amounts/values for two or more component(s), compounds(s), substituent(s) or parameters disclosed herein are thus also disclosed in combination with each other for the purposes of this description.

It is further understood that each range disclosed herein is to be interpreted as a disclosure of each specific value within the disclosed range that has the same number of significant digits. Thus, a range of from 1-4 is to be interpreted as an express disclosure of the values 1, 2, 3 and 4.

It is further understood that each lower limit of each range disclosed herein is to be interpreted as disclosed in combination with each upper limit of each range and each specific value within each range disclosed herein for the same component, compounds, substituent or parameter. Thus, this disclosure to be interpreted as a disclosure of all ranges derived by combining each lower limit of each range with each upper limit of each range or with each specific value within each range, or by combining each upper limit of each range with each specific value within each range.

Furthermore, specific amounts/values of a component, compound, substituent or parameter disclosed in the description or an example is to be interpreted as a disclosure of either a lower or an upper limit of a range and thus can be

32

combined with any other lower or upper limit of a range or specific amount/value for the same component, compound, substituent or parameter disclosed elsewhere in the application to form a range for that component, compound, substituent or parameter.

What is claimed is:

1. A method for reducing wear in an internal combustion engine of a hybrid vehicle comprising lubricating the internal combustion engine of the hybrid vehicle with a lubricating oil composition comprising:

greater than 50 wt. % of a base oil of lubricating viscosity; and

an amount of one or more zinc dialkyl dithiophosphate compound(s) sufficient to provide:

from 550 ppmw phosphorus to 710 ppmw phosphorus, based on a total weight of the lubricating oil composition, and

from 200 ppmw zinc to 821 ppmw zinc, based on the total weight of the lubricating oil composition; and

wherein the one or more zinc dialkyl dithiophosphate compounds are derived from 100 mole % of one or more primary alkyl alcohol(s),

the one or more zinc dialkyl dithiophosphate compound(s) has a zinc to phosphorus molar ratio of at least 1.20,

the lubricating oil composition further comprises one or more components selected from the group consisting of succinimide dispersant(s), borated succinimide dispersant(s), organic friction modifier(s), molybdenum-containing compound(s), calcium sulfonate detergent(s), antioxidant(s), antifoam agent(s), pour point depressant(s), and viscosity index improver(s), and the internal combustion engine of the hybrid vehicle is operated at a temperature of 100° C. or less.

2. The method of claim 1, wherein the one or more zinc dialkyl dithiophosphate compound(s) is derived from the one or more primary alkyl alcohol(s) having an alkyl group with 3 to 9 carbon atoms.

3. The method of claim 1, wherein the one or more zinc dialkyl dithiophosphate compound(s) comprises an average number of total carbon atoms per mole of phosphorus of from about 8 to about 30.

4. The method of claim 1, wherein the alkyl group of the one or more primary alkyl alcohol(s) has branching at the beta carbon relative to the hydroxyl group.

5. The method of claim 1, wherein the one or more zinc dialkyl dithiophosphate compound(s) is derived from the one or more primary alkyl alcohol(s) selected from the group consisting of n-propyl alcohol, isopropyl alcohol, n-butyl alcohol, 2-butanol, n-penyl alcohol, hexanol, methyl isobutyl carbinol, isohexanol, n-heptanol, isoheptanol, octanol, isobutyl alcohol, amyl alcohol, and 2-ethylhexanol.

6. The method of claim 1, wherein the one or more zinc dialkyl dithiophosphate compound(s) is derived from two or more primary alkyl alcohols.

7. The method of claim 1, wherein the one or more zinc dialkyl dithiophosphate compound(s) is overbased with zinc oxide.

8. The method of claim 1, wherein the lubricating oil composition further comprises a calcium-sulfonate detergent in an amount sufficient to provide from about 500 ppmw to about 2000 ppmw calcium to the lubricating oil composition, based on a total weight of the lubricating oil composition.

9. The method of claim 1, wherein the lubricating oil composition comprises a borated succinimide dispersant.

10. The method of claim 1, wherein the lubricating oil composition further comprises succinimide dispersant(s),

borated succinimide dispersant(s), organic friction modifier(s), molybdenum-containing compound(s) calcium sulfonate detergent(s), antioxidant(s), antifoam agent(s), pour point depressant(s), and viscosity index improver(s).

11. A lubricating oil composition for use in an internal combustion engine of a hybrid vehicle, comprising:  
greater than 50 wt. % of a base oil of lubricating viscosity;  
and  
an amount of one or more zinc dialkyl dithiophosphate compound(s) sufficient to provide:  
from 550 ppmw phosphorus to 710 ppmw phosphorus, based on a total weight of the lubricating oil composition, and  
from 200 ppmw zinc to 821 ppmw zinc, based on the total weight of the lubricating oil composition, and  
wherein the one or more zinc dialkyl dithiophosphate compounds are derived from 100 mole % of one or more primary alkyl alcohol(s),  
the one or more zinc dialkyl dithiophosphate compound(s) has a zinc to phosphorus molar ratio of at least 1.20,  
the lubricating oil composition further comprises one or more components selected from the group consisting of succinimide dispersant(s), borated succinimide dispersant(s), organic friction modifier(s), molybdenum-containing compound(s), calcium sulfonate detergent(s), antioxidant(s), antifoam agent(s), pour point depressant(s), and viscosity index improver(s), and  
the lubricating oil composition is formulated for use in an internal combustion engine of the hybrid vehicle which is operated at a temperature of 100° C. or less.

\* \* \* \* \*